



US009926763B2

(12) **United States Patent**  
**Mazyar et al.**

(10) **Patent No.:** **US 9,926,763 B2**  
(b4) **Date of Patent:** **Mar. 27, 2018**

(54) **CORRODIBLE DOWNHOLE ARTICLE AND METHOD OF REMOVING THE ARTICLE FROM DOWNHOLE ENVIRONMENT**

(71) Applicants: **Oleg A. Mazyar**, Houston, TX (US);  
**Matthew T. McCoy**, Richmond, TX (US)

(72) Inventors: **Oleg A. Mazyar**, Houston, TX (US);  
**Matthew T. McCoy**, Richmond, TX (US)

(73) Assignee: **BAKER HUGHES, A GE COMPANY, LLC**, Houston, TX (US)

(\*) Notice: Subject to any disclaimer, the term of this patent is extended or adjusted under 35 U.S.C. 154(b) by 0 days.

(21) Appl. No.: **14/826,710**

(22) Filed: **Aug. 14, 2015**

(65) **Prior Publication Data**

US 2015/0354312 A1 Dec. 10, 2015

**Related U.S. Application Data**

(62) Division of application No. 13/162,781, filed on Jun. 17, 2011, now Pat. No. 9,139,928.

(51) **Int. Cl.**  
**E21B 33/12** (2006.01)  
**C23C 18/16** (2006.01)  
**C25D 5/48** (2006.01)

(52) **U.S. Cl.**  
CPC ..... **E21B 33/12** (2013.01); **C23C 18/1637** (2013.01); **C23C 18/1689** (2013.01); **C25D 5/48** (2013.01)

(58) **Field of Classification Search**

None

See application file for complete search history.

(56) **References Cited**

U.S. PATENT DOCUMENTS

|               |         |                |
|---------------|---------|----------------|
| 1,468,905 A   | 9/1923  | Herman         |
| 2,189,697 A   | 2/1940  | Baker          |
| 2,222,233 A   | 11/1940 | Mize           |
| 2,225,143 A   | 12/1940 | Baker et al.   |
| 2,238,895 A   | 4/1941  | Gage           |
| 2,261,292 A * | 11/1941 | Salnikov ..... |
|               |         | E21B 29/02     |
|               |         | 166/291        |
| 2,294,648 A   | 9/1942  | Gerhard        |
| 2,301,624 A   | 11/1942 | Holt           |

(Continued)

FOREIGN PATENT DOCUMENTS

|    |            |        |
|----|------------|--------|
| CA | 2783241 A1 | 6/2011 |
| CA | 2783346 A1 | 6/2011 |

(Continued)

OTHER PUBLICATIONS

Adams, et al.; "Thermal stabilities of aromatic acids as geothermal tracers", Geothermics, vol. 21, No. 3, 1992, pp. 323-339.

(Continued)

Primary Examiner — Daniel J Schleis

(74) Attorney, Agent, or Firm — Cantor Colburn LLP

(57) **ABSTRACT**

A method of removing a corrodible downhole article having a surface coating includes eroding the surface coating by physical abrasion, chemical etching, or a combination of physical abrasion and chemical etching, the surface coating comprising a metallic layer of a metal resistant to corrosion by a corrosive material.

**20 Claims, 2 Drawing Sheets**



| (56)                  | References Cited |                                          |
|-----------------------|------------------|------------------------------------------|
| U.S. PATENT DOCUMENTS |                  |                                          |
| 2,352,993 A           | 7/1944           | Albertson                                |
| 2,394,843 A           | 2/1946           | Cooke et al.                             |
| 2,672,199 A           | 3/1954           | McKenna                                  |
| 2,753,941 A           | 7/1956           | Hebard et al.                            |
| 2,754,910 A           | 7/1956           | Derrick et al.                           |
| 2,933,136 A           | 4/1960           | Ayers et al.                             |
| 2,983,634 A           | 5/1961           | Budininkas et al.                        |
| 3,057,405 A           | 10/1962          | Mallinger                                |
| 3,066,391 A           | 12/1962          | Vordahl                                  |
| 3,106,959 A           | 10/1963          | Huitt et al.                             |
| 3,142,338 A           | 7/1964           | Brown                                    |
| 3,152,009 A           | 10/1964          | Delong                                   |
| 3,196,949 A           | 7/1965           | Thomas                                   |
| 3,242,988 A           | 3/1966           | McGuire et al.                           |
| 3,316,748 A           | 5/1967           | Lang et al.                              |
| 3,326,291 A           | 6/1967           | Zandmer et al.                           |
| 3,343,537 A           | 9/1967           | Graham                                   |
| 3,347,317 A           | 10/1967          | Solis                                    |
| 3,347,714 A           | 10/1967          | Broverman et al.                         |
| 3,390,724 A           | 7/1968           | Caldwell                                 |
| 3,395,758 A           | 8/1968           | Kelly et al.                             |
| 3,406,101 A           | 10/1968          | Kilpatrick                               |
| 3,416,918 A           | 12/1968          | Henry                                    |
| 3,465,181 A           | 9/1969           | Colby et al.                             |
| 3,489,218 A           | 1/1970           | Means                                    |
| 3,513,230 A           | 5/1970           | Rhees et al.                             |
| 3,602,305 A           | 8/1971           | Kisling                                  |
| 3,637,446 A           | 1/1972           | Elliott et al.                           |
| 3,645,331 A           | 2/1972           | Maurer et al.                            |
| 3,660,049 A           | 5/1972           | Benjamin                                 |
| 3,765,484 A           | 10/1973          | Hamby, Jr. et al.                        |
| 3,768,563 A           | 10/1973          | Blount                                   |
| 3,775,823 A           | 12/1973          | Adolph et al.                            |
| 3,816,080 A           | 6/1974           | Bomford et al.                           |
| 3,878,889 A           | 4/1975           | Seabourn                                 |
| 3,894,850 A           | 7/1975           | Kovalchuk et al.                         |
| 3,924,677 A           | 12/1975          | Prenner et al.                           |
| 4,010,583 A           | 3/1977           | Highberg                                 |
| 4,039,717 A           | 8/1977           | Titus                                    |
| 4,050,529 A           | 9/1977           | Tagirov et al.                           |
| 4,157,732 A           | 6/1979           | Fonner                                   |
| 4,248,307 A           | 2/1981           | Silberman et al.                         |
| 4,284,137 A           | 8/1981           | Taylor                                   |
| 4,292,377 A           | 9/1981           | Petersen et al.                          |
| 4,372,384 A           | 2/1983           | Kinney                                   |
| 4,373,584 A           | 2/1983           | Silberman et al.                         |
| 4,373,952 A           | 2/1983           | Parent                                   |
| 4,374,543 A           | 2/1983           | Richardson                               |
| 4,384,616 A           | 5/1983           | Dellinger                                |
| 4,395,440 A           | 7/1983           | Abe et al.                               |
| 4,399,871 A           | 8/1983           | Adkins et al.                            |
| 4,407,368 A           | 10/1983          | Erbstoesser                              |
| 4,422,508 A           | 12/1983          | Rutledge, Jr. et al.                     |
| 4,452,311 A           | 6/1984           | Speegle et al.                           |
| 4,475,729 A           | 10/1984          | Costigan                                 |
| 4,498,543 A           | 2/1985           | Pye et al.                               |
| 4,499,048 A           | 2/1985           | Hanejko                                  |
| 4,499,049 A           | 2/1985           | Hanejko                                  |
| 4,524,825 A           | 6/1985           | Fore                                     |
| 4,526,840 A           | 7/1985           | Jerabek                                  |
| 4,534,414 A           | 8/1985           | Pringle                                  |
| 4,539,175 A           | 9/1985           | Lichti et al.                            |
| 4,554,986 A           | 11/1985          | Jones                                    |
| 4,619,699 A           | 10/1986          | Petkovic-Luton et al.                    |
| 4,640,354 A           | 2/1987           | Boisson                                  |
| 4,664,962 A           | 5/1987           | Desmarais, Jr.                           |
| 4,668,470 A           | 5/1987           | Gilman et al.                            |
| 4,673,549 A           | 6/1987           | Ecer                                     |
| 4,674,572 A           | 6/1987           | Gallus                                   |
| 4,678,037 A           | 7/1987           | Smith                                    |
| 4,681,133 A           | 7/1987           | Weston                                   |
| 4,688,641 A           | 8/1987           | Knieriemen                               |
| 4,690,796 A           | 9/1987           | Paliwal                                  |
| 4,693,863 A           | 9/1987           | Del Corso et al.                         |
| 4,703,807 A           | 11/1987          | Weston                                   |
|                       |                  | 4,706,753 A 11/1987 Ohkochi et al.       |
|                       |                  | 4,708,202 A 11/1987 Sukup et al.         |
|                       |                  | 4,708,208 A 11/1987 Halbardier           |
|                       |                  | 4,709,761 A 12/1987 Setterberg, Jr.      |
|                       |                  | 4,714,116 A 12/1987 Brunner              |
|                       |                  | 4,716,964 A 1/1988 Erbstoesser et al.    |
|                       |                  | 4,719,971 A 1/1988 Owens                 |
|                       |                  | 4,721,159 A 1/1988 Ohkochi et al.        |
|                       |                  | 4,738,599 A 4/1988 Shilling              |
|                       |                  | 4,741,973 A 5/1988 Condit et al.         |
|                       |                  | 4,768,588 A 9/1988 Kupsa                 |
|                       |                  | 4,775,598 A 10/1988 Jaeckel              |
|                       |                  | 4,784,226 A 11/1988 Wyatt                |
|                       |                  | 4,805,699 A 2/1989 Halbardier            |
|                       |                  | 4,817,725 A 4/1989 Jenkins               |
|                       |                  | 4,834,184 A 5/1989 Streich et al.        |
|                       |                  | H635 H 6/1989 Johnson et al.             |
|                       |                  | 4,850,432 A 7/1989 Porter et al.         |
|                       |                  | 4,853,056 A 8/1989 Hoffman               |
|                       |                  | 4,869,324 A 9/1989 Holder                |
|                       |                  | 4,869,325 A 9/1989 Halbardier            |
|                       |                  | 4,880,059 A 11/1989 Brandell et al.      |
|                       |                  | 4,889,187 A 12/1989 Terrell et al.       |
|                       |                  | 4,890,675 A 1/1990 Dew                   |
|                       |                  | 4,901,794 A 2/1990 Baugh et al.          |
|                       |                  | 4,909,320 A 3/1990 Hebert et al.         |
|                       |                  | 4,929,415 A 5/1990 Okazaki               |
|                       |                  | 4,932,474 A 6/1990 Schroeder, Jr. et al. |
|                       |                  | 4,938,309 A 7/1990 Emdy                  |
|                       |                  | 4,944,351 A 7/1990 Eriksen et al.        |
|                       |                  | 4,949,788 A 8/1990 Szarka et al.         |
|                       |                  | 4,952,902 A 8/1990 Kawaguchi et al.      |
|                       |                  | 4,975,412 A 12/1990 Okazaki et al.       |
|                       |                  | 4,977,958 A 12/1990 Miller               |
|                       |                  | 4,981,177 A 1/1991 Carmody et al.        |
|                       |                  | 4,986,361 A 1/1991 Mueller et al.        |
|                       |                  | 4,997,622 A 3/1991 Regazzoni et al.      |
|                       |                  | 5,006,044 A 4/1991 Walker, Sr. et al.    |
|                       |                  | 5,010,955 A 4/1991 Springer              |
|                       |                  | 5,036,921 A 8/1991 Pittard et al.        |
|                       |                  | 5,048,611 A 9/1991 Cochran               |
|                       |                  | 5,049,165 A 9/1991 Tselesin              |
|                       |                  | 5,061,323 A 10/1991 Deluccia             |
|                       |                  | 5,063,775 A 11/1991 Walker, Sr. et al.   |
|                       |                  | 5,073,207 A 12/1991 Faure et al.         |
|                       |                  | 5,074,361 A 12/1991 Brisco et al.        |
|                       |                  | 5,076,869 A 12/1991 Bourell et al.       |
|                       |                  | 5,084,088 A 1/1992 Okazaki               |
|                       |                  | 5,087,304 A 2/1992 Chang et al.          |
|                       |                  | 5,090,480 A 2/1992 Pittard et al.        |
|                       |                  | 5,095,988 A 3/1992 Bode                  |
|                       |                  | 5,103,911 A 4/1992 Heijnen               |
|                       |                  | 5,117,915 A 6/1992 Mueller et al.        |
|                       |                  | 5,161,614 A 11/1992 Wu et al.            |
|                       |                  | 5,171,734 A 12/1992 Sanjurjo et al.      |
|                       |                  | 5,178,216 A 1/1993 Giroux et al.         |
|                       |                  | 5,181,571 A 1/1993 Mueller et al.        |
|                       |                  | 5,183,631 A 2/1993 Kugimiya et al.       |
|                       |                  | 5,188,182 A 2/1993 Echols, III et al.    |
|                       |                  | 5,188,183 A 2/1993 Hopmann et al.        |
|                       |                  | 5,204,055 A 4/1993 Sachs et al.          |
|                       |                  | 5,222,867 A 6/1993 Walker, Sr. et al.    |
|                       |                  | 5,226,483 A 7/1993 Williamson, Jr.       |
|                       |                  | 5,228,518 A 7/1993 Wilson et al.         |
|                       |                  | 5,234,055 A 8/1993 Cornette              |
|                       |                  | 5,252,365 A 10/1993 White                |
|                       |                  | 5,253,714 A 10/1993 Davis et al.         |
|                       |                  | 5,271,468 A 12/1993 Streich et al.       |
|                       |                  | 5,282,509 A 2/1994 Schurr, III           |
|                       |                  | 5,292,478 A 3/1994 Scorey                |
|                       |                  | 5,293,940 A 3/1994 Hromas et al.         |
|                       |                  | 5,304,260 A 4/1994 Aikawa et al.         |
|                       |                  | 5,304,588 A 4/1994 Boysen et al.         |
|                       |                  | 5,309,874 A 5/1994 Willermet et al.      |
|                       |                  | 5,310,000 A 5/1994 Arterbury et al.      |
|                       |                  | 5,316,598 A 5/1994 Chang et al.          |
|                       |                  | 5,318,746 A 6/1994 Lashmore              |
|                       |                  | 5,325,522 A 10/1994 Kugimiya et al.      |
|                       |                  | 5,380,473 A 1/1995 Bogue et al.          |

(56)

## References Cited

## U.S. PATENT DOCUMENTS

|             |         |                    |              |         |                    |
|-------------|---------|--------------------|--------------|---------|--------------------|
| 5,387,380 A | 2/1995  | Cima et al.        | 6,085,837 A  | 7/2000  | Massinon et al.    |
| 5,392,860 A | 2/1995  | Ross               | 6,095,247 A  | 8/2000  | Streich et al.     |
| 5,394,236 A | 2/1995  | Murnick            | 6,119,783 A  | 9/2000  | Parker et al.      |
| 5,394,941 A | 3/1995  | Venditto et al.    | 6,142,237 A  | 11/2000 | Christmas et al.   |
| 5,398,754 A | 3/1995  | Dinhobole          | 6,161,622 A  | 12/2000 | Robb               |
| 5,407,011 A | 4/1995  | Layton             | 6,167,970 B1 | 1/2001  | Stout et al.       |
| 5,409,555 A | 4/1995  | Fujita et al.      | 6,170,583 B1 | 1/2001  | Boyce              |
| 5,411,082 A | 5/1995  | Kennedy            | 6,173,779 B1 | 1/2001  | Smith              |
| 5,417,285 A | 5/1995  | Van Buskirk et al. | 6,176,323 B1 | 1/2001  | Weirich et al.     |
| 5,425,424 A | 6/1995  | Reinhardt et al.   | 6,189,616 B1 | 2/2001  | Gano et al.        |
| 5,427,177 A | 6/1995  | Jordan, Jr. et al. | 6,189,618 B1 | 2/2001  | Beeman et al.      |
| 5,435,392 A | 7/1995  | Kennedy            | 6,213,202 B1 | 4/2001  | Read, Jr.          |
| 5,439,051 A | 8/1995  | Kennedy et al.     | 6,220,350 B1 | 4/2001  | Brothers et al.    |
| 5,454,430 A | 10/1995 | Kennedy et al.     | 6,220,357 B1 | 4/2001  | Carmichael et al.  |
| 5,456,317 A | 10/1995 | Hood, III et al.   | 6,228,904 B1 | 5/2001  | Yadav et al.       |
| 5,456,327 A | 10/1995 | Denton et al.      | 6,237,688 B1 | 5/2001  | Burleson et al.    |
| 5,464,062 A | 11/1995 | Blizzard, Jr.      | 6,238,280 B1 | 5/2001  | Ritt et al.        |
| 5,472,048 A | 12/1995 | Kennedy et al.     | 6,241,021 B1 | 6/2001  | Bowling            |
| 5,474,131 A | 12/1995 | Jordan, Jr. et al. | 6,248,399 B1 | 6/2001  | Hehmann            |
| 5,477,923 A | 12/1995 | Jordan, Jr. et al. | 6,250,392 B1 | 6/2001  | Muth               |
| 5,479,986 A | 1/1996  | Gano et al.        | 6,261,432 B1 | 7/2001  | Huber et al.       |
| 5,506,055 A | 4/1996  | Dorfman et al.     | 6,273,187 B1 | 8/2001  | Voisin, Jr. et al. |
| 5,507,439 A | 4/1996  | Story              | 6,276,452 B1 | 8/2001  | Davis et al.       |
| 5,511,620 A | 4/1996  | Baugh et al.       | 6,276,457 B1 | 8/2001  | Moffatt et al.     |
| 5,524,699 A | 6/1996  | Cook               | 6,279,656 B1 | 8/2001  | Sinclair et al.    |
| 5,526,880 A | 6/1996  | Jordan, Jr. et al. | 6,287,445 B1 | 9/2001  | Lashmore et al.    |
| 5,526,881 A | 6/1996  | Martin et al.      | 6,302,205 B1 | 10/2001 | Ryll               |
| 5,529,746 A | 6/1996  | Knoss et al.       | 6,315,041 B1 | 11/2001 | Carlisle et al.    |
| 5,533,573 A | 7/1996  | Jordan, Jr. et al. | 6,315,050 B2 | 11/2001 | Vaynshteyn et al.  |
| 5,536,485 A | 7/1996  | Kume et al.        | 6,325,148 B1 | 12/2001 | Trahan et al.      |
| 5,558,153 A | 9/1996  | Holcombe et al.    | 6,328,110 B1 | 12/2001 | Joubert            |
| 5,601,924 A | 2/1997  | Beane              | 6,341,653 B1 | 1/2002  | Firmaniuk et al.   |
| 5,607,017 A | 3/1997  | Owens et al.       | 6,341,747 B1 | 1/2002  | Schmidt et al.     |
| 5,623,993 A | 4/1997  | Van Buskirk et al. | 6,349,766 B1 | 2/2002  | Bussear et al.     |
| 5,623,994 A | 4/1997  | Robinson           | 6,354,372 B1 | 3/2002  | Carisella et al.   |
| 5,636,691 A | 6/1997  | Hendrickson et al. | 6,354,379 B2 | 3/2002  | Miszewski et al.   |
| 5,641,023 A | 6/1997  | Ross et al.        | 6,357,322 B1 | 3/2002  | Dolan et al.       |
| 5,647,444 A | 7/1997  | Williams           | 6,357,332 B1 | 3/2002  | Vecchio            |
| 5,665,289 A | 9/1997  | Chung et al.       | 6,371,206 B1 | 4/2002  | Mills              |
| 5,677,372 A | 10/1997 | Yamamoto et al.    | 6,372,346 B1 | 4/2002  | Toth               |
| 5,685,372 A | 11/1997 | Gano               | 6,382,244 B2 | 5/2002  | Vann               |
| 5,701,576 A | 12/1997 | Fujita et al.      | 6,390,195 B1 | 5/2002  | Nguyen et al.      |
| 5,707,214 A | 1/1998  | Schmidt            | 6,390,200 B1 | 5/2002  | Allamon et al.     |
| 5,709,269 A | 1/1998  | Head               | 6,394,180 B1 | 5/2002  | Berscheidt et al.  |
| 5,720,344 A | 2/1998  | Newman             | 6,394,185 B1 | 5/2002  | Constien           |
| 5,728,195 A | 3/1998  | Eastman et al.     | 6,395,402 B1 | 5/2002  | Lambert et al.     |
| 5,765,639 A | 6/1998  | Muth               | 6,397,950 B1 | 6/2002  | Streich et al.     |
| 5,772,735 A | 6/1998  | Sehgal et al.      | 6,401,547 B1 | 6/2002  | Hatfield et al.    |
| 5,782,305 A | 7/1998  | Hicks              | 6,403,210 B1 | 6/2002  | Stuivinga et al.   |
| 5,797,454 A | 8/1998  | Hipp               | 6,408,946 B1 | 6/2002  | Marshall et al.    |
| 5,826,652 A | 10/1998 | Tapp               | 6,419,023 B1 | 7/2002  | George et al.      |
| 5,826,661 A | 10/1998 | Parker et al.      | 6,439,313 B1 | 8/2002  | Thomeer et al.     |
| 5,829,520 A | 11/1998 | Johnson            | 6,446,717 B1 | 9/2002  | White et al.       |
| 5,836,396 A | 11/1998 | Norman             | 6,457,525 B1 | 10/2002 | Scott              |
| 5,857,521 A | 1/1999  | Ross et al.        | 6,467,546 B2 | 10/2002 | Allamon et al.     |
| 5,881,816 A | 3/1999  | Wright             | 6,470,965 B1 | 10/2002 | Winzer             |
| 5,896,819 A | 4/1999  | Turila et al.      | 6,491,097 B1 | 12/2002 | Oneal et al.       |
| 5,902,424 A | 5/1999  | Fujita et al.      | 6,491,116 B2 | 12/2002 | Berscheidt et al.  |
| 5,934,372 A | 8/1999  | Muth               | 6,513,598 B2 | 2/2003  | Moore et al.       |
| 5,941,309 A | 8/1999  | Appleton           | 6,513,600 B2 | 2/2003  | Ross               |
| 5,960,881 A | 10/1999 | Allamon et al.     | 6,540,033 B1 | 4/2003  | Sullivan et al.    |
| 5,985,466 A | 11/1999 | Atarashi et al.    | 6,543,543 B2 | 4/2003  | Muth               |
| 5,988,287 A | 11/1999 | Jordan, Jr. et al. | 6,561,275 B2 | 5/2003  | Glass et al.       |
| 5,990,051 A | 11/1999 | Ischy et al.       | 6,588,507 B2 | 7/2003  | Dusterhoft et al.  |
| 5,992,452 A | 11/1999 | Nelson, II         | 6,591,915 B2 | 7/2003  | Burriss et al.     |
| 5,992,520 A | 11/1999 | Schultz et al.     | 6,601,648 B2 | 8/2003  | Ebinger            |
| 6,007,314 A | 12/1999 | Nelson, II         | 6,601,650 B2 | 8/2003  | Sundararajan       |
| 6,024,915 A | 2/2000  | Kume et al.        | 6,609,569 B2 | 8/2003  | Howlett et al.     |
| 6,032,735 A | 3/2000  | Echols             | 6,612,826 B1 | 9/2003  | Bauer et al.       |
| 6,036,777 A | 3/2000  | Sachs              | 6,613,383 B1 | 9/2003  | George et al.      |
| 6,047,773 A | 4/2000  | Zeltmann et al.    | 6,619,400 B2 | 9/2003  | Brunet             |
| 6,050,340 A | 4/2000  | Scott              | 6,634,428 B2 | 10/2003 | Krauss et al.      |
| 6,069,313 A | 5/2000  | Kay                | 6,662,886 B2 | 12/2003 | Russell            |
| 6,076,600 A | 6/2000  | Vick, Jr. et al.   | 6,675,889 B1 | 1/2004  | Mullins et al.     |
| 6,079,496 A | 6/2000  | Hirth              | 6,699,305 B2 | 3/2004  | Myrick             |
|             |         |                    | 6,712,153 B2 | 3/2004  | Turley et al.      |
|             |         |                    | 6,712,797 B1 | 3/2004  | Southern, Jr.      |
|             |         |                    | 6,713,177 B2 | 3/2004  | George et al.      |
|             |         |                    | 6,715,541 B2 | 4/2004  | Pedersen et al.    |

| (56)                  | References Cited             |              |                                 |  |
|-----------------------|------------------------------|--------------|---------------------------------|--|
| U.S. PATENT DOCUMENTS |                              |              |                                 |  |
| 6,719,051 B2          | 4/2004 Hailey, Jr. et al.    | 7,331,388 B2 | 2/2008 Vilela et al.            |  |
| 6,755,249 B2          | 6/2004 Robison et al.        | 7,337,854 B2 | 3/2008 Horn et al.              |  |
| 6,769,491 B2          | 8/2004 Zimmerman et al.      | 7,346,456 B2 | 3/2008 Le Bemadjiel             |  |
| 6,776,228 B2          | 8/2004 Pedersen et al.       | 7,350,582 B2 | 4/2008 McKeachnie et al.        |  |
| 6,779,599 B2          | 8/2004 Mullins et al.        | 7,353,879 B2 | 4/2008 Todd et al.              |  |
| 6,799,638 B2          | 10/2004 Butterfield, Jr.     | 7,360,593 B2 | 4/2008 Constien                 |  |
| 6,810,960 B2          | 11/2004 Pia                  | 7,360,597 B2 | 4/2008 Blaisdell                |  |
| 6,817,414 B2          | 11/2004 Lee                  | 7,363,970 B2 | 4/2008 Corre et al.             |  |
| 6,831,044 B2          | 12/2004 Constien             | 7,373,978 B2 | 5/2008 Barry et al.             |  |
| 6,883,611 B2          | 4/2005 Smith et al.          | 7,384,443 B2 | 6/2008 Mirchandani              |  |
| 6,887,297 B2          | 5/2005 Winter et al.         | 7,387,158 B2 | 6/2008 Murray et al.            |  |
| 6,896,049 B2          | 5/2005 Moyes                 | 7,387,165 B2 | 6/2008 Lopez De Cardenas et al. |  |
| 6,896,061 B2          | 5/2005 Hriscu et al.         | 7,392,841 B2 | 7/2008 Murray et al.            |  |
| 6,899,176 B2          | 5/2005 Hailey, Jr. et al.    | 7,401,648 B2 | 7/2008 Bennett                  |  |
| 6,899,777 B2          | 5/2005 Vaidyanathan et al.   | 7,416,029 B2 | 8/2008 Telfer et al.            |  |
| 6,908,516 B2          | 6/2005 Hehmann et al.        | 7,422,058 B2 | 9/2008 O'Malley                 |  |
| 6,913,827 B2          | 7/2005 George et al.         | 7,426,964 B2 | 9/2008 Lynde et al.             |  |
| 6,926,086 B2          | 8/2005 Patterson et al.      | 7,441,596 B2 | 10/2008 Wood et al.             |  |
| 6,932,159 B2          | 8/2005 Hovem                 | 7,445,049 B2 | 11/2008 Howard et al.           |  |
| 6,939,388 B2          | 9/2005 Angeliu               | 7,451,815 B2 | 11/2008 Hailey, Jr.             |  |
| 6,945,331 B2          | 9/2005 Patel                 | 7,451,817 B2 | 11/2008 Reddy et al.            |  |
| 6,951,331 B2          | 10/2005 Haughom et al.       | 7,503,390 B2 | 3/2009 Badalamenti et al.       |  |
| 6,959,759 B2          | 11/2005 Doane et al.         | 7,503,399 B2 | 3/2009 Turng et al.             |  |
| 6,973,970 B2          | 12/2005 Johnston et al.      | 7,509,993 B1 | 3/2009 Williamson et al.        |  |
| 6,973,973 B2          | 12/2005 Howard et al.        | 7,510,018 B2 | 4/2009 Gramstad et al.          |  |
| 6,983,796 B2          | 1/2006 Bayne et al.          | 7,513,311 B2 | 5/2009 Huang et al.             |  |
| 6,986,390 B2          | 1/2006 Doane et al.          | 7,527,103 B2 | 5/2009 Wardle et al.            |  |
| 7,013,989 B2          | 3/2006 Hammond et al.        | 7,537,825 B1 | 6/2009 Murray et al.            |  |
| 7,013,998 B2          | 3/2006 Ray et al.            | 7,552,777 B2 | 6/2009 Murray                   |  |
| 7,017,664 B2          | 3/2006 Walker et al.         | 7,552,779 B2 | 7/2009 Clem                     |  |
| 7,017,677 B2          | 3/2006 Keshavan et al.       | 7,559,357 B2 | 8/2009 East, Jr. et al.         |  |
| 7,021,389 B2          | 4/2006 Bishop et al.         | 7,575,062 B2 | 8/2009 Maloney et al.           |  |
| 7,025,146 B2          | 4/2006 King et al.           | 7,579,087 B2 | 9/2009 Tilghman                 |  |
| 7,028,778 B2          | 4/2006 Krywitsky             | 7,591,318 B2 | 10/2009 Slup et al.             |  |
| 7,044,230 B2          | 5/2006 Starr et al.          | 7,600,572 B2 | 10/2009 Vaidya et al.           |  |
| 7,049,272 B2          | 5/2006 Sinclair et al.       | 7,604,049 B2 | 10/2009 Richard et al.          |  |
| 7,051,805 B2          | 5/2006 Doane et al.          | 7,604,055 B2 | 10/2009 Tom et al.              |  |
| 7,059,410 B2          | 6/2006 Bousche et al.        | 7,607,476 B2 | 11/2009 Surjaatmadja et al.     |  |
| 7,090,027 B1          | 8/2006 Williams              | 7,617,871 B2 | 12/2009 Goldberg et al.         |  |
| 7,093,664 B2          | 8/2006 Todd et al.           | 7,635,023 B2 | 1/2010 Phi et al.               |  |
| 7,096,945 B2          | 8/2006 Richards et al.       | 7,640,988 B2 | 2/2010 Al-Anazi                 |  |
| 7,096,946 B2          | 8/2006 Jasser et al.         | 7,661,480 B2 | 2/2010 Todd et al.              |  |
| 7,097,807 B1          | 8/2006 Meeks, III et al.     | 7,661,481 B2 | 2/2010 Patel et al.             |  |
| 7,097,906 B2          | 8/2006 Gardner               | 7,665,537 B2 | 2/2010 Buyers et al.            |  |
| 7,108,080 B2          | 9/2006 Tessari et al.        | 7,686,082 B2 | 3/2010 Marsh                    |  |
| 7,111,682 B2          | 9/2006 Blaisdell             | 7,690,436 B2 | 4/2010 Turley et al.            |  |
| 7,128,145 B2          | 10/2006 Mickey               | 7,699,101 B2 | 4/2010 Fripp et al.             |  |
| 7,141,207 B2          | 11/2006 Jandeska, Jr. et al. | 7,703,510 B2 | 4/2010 Xu                       |  |
| 7,150,326 B2          | 12/2006 Bishop et al.        | 7,703,511 B2 | 4/2010 Stoesz                   |  |
| 7,163,066 B2          | 1/2007 Lehr                  | 7,708,078 B2 | 5/2010 Jones et al.             |  |
| 7,165,622 B2          | 1/2007 Hirth et al.          | 7,709,421 B2 | 5/2010 Loretz et al.            |  |
| 7,168,494 B2          | 1/2007 Starr et al.          | 7,712,541 B2 | 5/2010 Crews et al.             |  |
| 7,174,963 B2          | 2/2007 Bertelsen             | 7,723,272 B2 | 6/2010 Xu                       |  |
| 7,182,135 B2          | 2/2007 Szarka                | 7,726,406 B2 | 6/2010 Loehr et al.             |  |
| 7,188,559 B1          | 3/2007 Vecchio               | 7,735,578 B2 | 6/2010 Cook et al.              |  |
| 7,210,527 B2          | 5/2007 Walker et al.         | 7,743,836 B2 | 7/2010 Loehr                    |  |
| 7,210,533 B2          | 5/2007 Starr et al.          | 7,752,971 B2 | 7/2010 Rytlewski                |  |
| 7,217,311 B2          | 5/2007 Hong et al.           | 7,757,773 B2 | 7/2010 Richard et al.           |  |
| 7,234,530 B2          | 6/2007 Gass                  | 7,762,342 B2 | 8/2010 Barnett                  |  |
| 7,250,188 B2          | 7/2007 Dodelet et al.        | 7,770,652 B2 | 8/2010 Palumbo et al.           |  |
| 7,252,162 B2          | 8/2007 Akinlade et al.       | 7,771,289 B2 | 8/2010 Richards et al.          |  |
| 7,255,172 B2          | 8/2007 Johnson               | 7,775,284 B2 | 8/2010 Surjaatmadja et al.      |  |
| 7,255,178 B2          | 8/2007 Slup et al.           | 7,775,285 B2 | 8/2010 Duphorne                 |  |
| 7,264,060 B2          | 9/2007 Wills                 | 7,775,286 B2 | 8/2010 Johnson                  |  |
| 7,267,172 B2          | 9/2007 Hofman                | 7,784,543 B2 | 9/2010 Johnson                  |  |
| 7,267,178 B2          | 9/2007 Krywitsky             | 7,793,714 B2 | 9/2010 Johnson                  |  |
| 7,270,186 B2          | 9/2007 Johnson               | 7,793,820 B2 | 9/2010 Hirano et al.            |  |
| 7,287,592 B2          | 10/2007 Surjaatmadja et al.  | 7,798,225 B2 | 9/2010 Giroux et al.            |  |
| 7,311,152 B2          | 12/2007 Howard et al.        | 7,798,226 B2 | 9/2010 Themig                   |  |
| 7,316,274 B2          | 1/2008 Xu et al.             | 7,798,236 B2 | 9/2010 McKeachnie et al.        |  |
| 7,320,365 B2          | 1/2008 Pia                   | 7,806,189 B2 | 10/2010 Frazier                 |  |
| 7,322,412 B2          | 1/2008 Badalamenti et al.    | 7,806,192 B2 | 10/2010 Foster et al.           |  |
| 7,322,417 B2          | 1/2008 Rytlewski et al.      | 7,810,553 B2 | 10/2010 Cruickshank et al.      |  |
| 7,325,617 B2          | 2/2008 Murray                | 7,810,567 B2 | 10/2010 Daniels et al.          |  |
| 7,328,750 B2          | 2/2008 Swor et al.           | 7,819,198 B2 | 10/2010 Birckhead et al.        |  |

| (56)                  | References Cited           |                 |                               |  |  |  |  |
|-----------------------|----------------------------|-----------------|-------------------------------|--|--|--|--|
| U.S. PATENT DOCUMENTS |                            |                 |                               |  |  |  |  |
| 7,828,055 B2          | 11/2010 Willauer et al.    | 2002/0108756 A1 | 8/2002 Harrall et al.         |  |  |  |  |
| 7,833,944 B2          | 11/2010 Munoz et al.       | 2002/0136904 A1 | 9/2002 Glass et al.           |  |  |  |  |
| 7,849,927 B2          | 12/2010 Herrera            | 2002/0139541 A1 | 10/2002 Sheffield et al.      |  |  |  |  |
| 7,851,016 B2          | 12/2010 Arbab et al.       | 2002/0162661 A1 | 11/2002 Krauss et al.         |  |  |  |  |
| 7,855,168 B2          | 12/2010 Fuller et al.      | 2003/0019639 A1 | 1/2003 MacKay                 |  |  |  |  |
| 7,861,779 B2          | 1/2011 Vestavik            | 2003/0037925 A1 | 2/2003 Walker et al.          |  |  |  |  |
| 7,861,781 B2          | 1/2011 D'Arcy              | 2003/0060374 A1 | 3/2003 Cooke, Jr.             |  |  |  |  |
| 7,874,365 B2          | 1/2011 East, Jr. et al.    | 2003/0075326 A1 | 4/2003 Ebinger                |  |  |  |  |
| 7,878,253 B2          | 2/2011 Stowe et al.        | 2003/0104147 A1 | 6/2003 Bretschneider et al.   |  |  |  |  |
| 7,896,091 B2          | 3/2011 Williamson et al.   | 2003/0111728 A1 | 6/2003 Thai et al.            |  |  |  |  |
| 7,897,063 B1          | 3/2011 Perry et al.        | 2003/0127013 A1 | 7/2003 Zavitsanos et al.      |  |  |  |  |
| 7,900,696 B1          | 3/2011 Nish et al.         | 2003/0141060 A1 | 7/2003 Hailey et al.          |  |  |  |  |
| 7,900,703 B2          | 3/2011 Clark et al.        | 2003/0141061 A1 | 7/2003 Hailey et al.          |  |  |  |  |
| 7,909,096 B2          | 3/2011 Clark et al.        | 2003/0141079 A1 | 7/2003 Doane et al.           |  |  |  |  |
| 7,909,104 B2          | 3/2011 Bjorgum             | 2003/0150614 A1 | 8/2003 Brown et al.           |  |  |  |  |
| 7,909,110 B2          | 3/2011 Sharma et al.       | 2003/0155114 A1 | 8/2003 Pedersen et al.        |  |  |  |  |
| 7,909,115 B2          | 3/2011 Grove et al.        | 2003/0155115 A1 | 8/2003 Pedersen et al.        |  |  |  |  |
| 7,913,765 B2          | 3/2011 Crow et al.         | 2003/0159828 A1 | 8/2003 Howard et al.          |  |  |  |  |
| 7,918,275 B2          | 4/2011 Clem                | 2003/0164237 A1 | 9/2003 Butterfield            |  |  |  |  |
| 7,931,093 B2          | 4/2011 Foster et al.       | 2003/0183391 A1 | 10/2003 Hriscu et al.         |  |  |  |  |
| 7,938,191 B2          | 5/2011 Vaidya              | 2003/0226668 A1 | 12/2003 Zimmerman et al.      |  |  |  |  |
| 7,946,335 B2          | 5/2011 Bewlwy et al.       | 2004/0005483 A1 | 1/2004 Lin                    |  |  |  |  |
| 7,946,340 B2          | 5/2011 Surjaatmadja et al. | 2004/0020832 A1 | 2/2004 Richards et al.        |  |  |  |  |
| 7,958,940 B2          | 6/2011 Jameson             | 2004/0031605 A1 | 2/2004 Mickey                 |  |  |  |  |
| 7,963,331 B2          | 6/2011 Surjaatmadja et al. | 2004/0045723 A1 | 3/2004 Slup et al.            |  |  |  |  |
| 7,963,340 B2          | 6/2011 Gramstad et al.     | 2004/0055758 A1 | 3/2004 Brezinski et al.       |  |  |  |  |
| 7,963,342 B2          | 6/2011 George              | 2004/0058167 A1 | 3/2004 Arbab et al.           |  |  |  |  |
| 7,980,300 B2          | 7/2011 Roberts et al.      | 2004/0069502 A1 | 4/2004 Luke                   |  |  |  |  |
| 7,987,906 B1          | 8/2011 Troy                | 2004/0089449 A1 | 5/2004 Walton et al.          |  |  |  |  |
| 7,992,763 B2          | 8/2011 Vecchio et al.      | 2004/0094297 A1 | 5/2004 Malone et al.          |  |  |  |  |
| 8,020,619 B1          | 9/2011 Robertson et al.    | 2004/0145806 A1 | 8/2004 Bode et al.            |  |  |  |  |
| 8,020,620 B2          | 9/2011 Daniels et al.      | 2004/0159428 A1 | 8/2004 Hammond et al.         |  |  |  |  |
| 8,025,104 B2          | 9/2011 Cooke, Jr.          | 2004/0159446 A1 | 8/2004 Haugen et al.          |  |  |  |  |
| 8,028,767 B2          | 10/2011 Radford et al.     | 2004/0182583 A1 | 9/2004 Doane et al.           |  |  |  |  |
| 8,033,331 B2          | 10/2011 Themig             | 2004/0216868 A1 | 11/2004 Owen, Sr.             |  |  |  |  |
| 8,039,422 B1          | 10/2011 Al-Zahrani         | 2004/0231845 A1 | 11/2004 Cooke, Jr.            |  |  |  |  |
| 8,056,628 B2          | 11/2011 Whitsitt et al.    | 2004/0251025 A1 | 12/2004 Giroux et al.         |  |  |  |  |
| 8,056,638 B2          | 11/2011 Clayton et al.     | 2004/0256109 A1 | 12/2004 Johnson               |  |  |  |  |
| 8,109,340 B2          | 2/2012 Doane et al.        | 2004/0265157 A1 | 12/2004 Tessari et al.        |  |  |  |  |
| 8,127,856 B1          | 3/2012 Nish et al.         | 2004/0261993 A1 | 12/2004 Nguyen                |  |  |  |  |
| 8,153,052 B2          | 4/2012 Jackson et al.      | 2004/0261994 A1 | 12/2004 Nguyen et al.         |  |  |  |  |
| 8,163,060 B2          | 4/2012 Imanishi et al.     | 2005/0034876 A1 | 2/2005 Doane et al.           |  |  |  |  |
| 8,211,247 B2          | 7/2012 Marya et al.        | 2005/0051329 A1 | 3/2005 Blaisdell              |  |  |  |  |
| 8,211,248 B2          | 7/2012 Marya               | 2005/0064247 A1 | 3/2005 Sane                   |  |  |  |  |
| 8,226,740 B2          | 7/2012 Chaumonnot et al.   | 2005/0069449 A1 | 3/2005 Jackson et al.         |  |  |  |  |
| 8,230,731 B2          | 7/2012 Dyer et al.         | 2005/0074612 A1 | 4/2005 Eklund et al.          |  |  |  |  |
| 8,231,947 B2          | 7/2012 Vaidya et al.       | 2005/0098313 A1 | 5/2005 Atkins et al.          |  |  |  |  |
| 8,263,178 B2          | 9/2012 Boulos et al.       | 2005/0102255 A1 | 5/2005 Bultman                |  |  |  |  |
| 8,276,670 B2          | 10/2012 Patel              | 2005/0106316 A1 | 5/2005 Rigney et al.          |  |  |  |  |
| 8,277,974 B2          | 10/2012 Kumar et al.       | 2005/0126334 A1 | 6/2005 Mirchandani            |  |  |  |  |
| 8,297,364 B2          | 10/2012 Agrawal et al.     | 2005/0161212 A1 | 7/2005 Leismer et al.         |  |  |  |  |
| 8,327,931 B2          | 12/2012 Agrawal et al.     | 2005/0161224 A1 | 7/2005 Starr et al.           |  |  |  |  |
| 8,403,037 B2          | 3/2013 Agrawal et al.      | 2005/0165149 A1 | 7/2005 Chanak et al.          |  |  |  |  |
| 8,413,727 B2          | 4/2013 Holmes              | 2005/0194143 A1 | 9/2005 Xu et al.              |  |  |  |  |
| 8,425,651 B2          | 4/2013 Xu et al.           | 2005/0199401 A1 | 9/2005 Patel et al.           |  |  |  |  |
| 8,459,347 B2          | 6/2013 Stout               | 2005/0205264 A1 | 9/2005 Starr et al.           |  |  |  |  |
| 8,490,689 B1          | 7/2013 McClinton et al.    | 2005/0205265 A1 | 9/2005 Todd et al.            |  |  |  |  |
| 8,535,604 B1          | 9/2013 Baker et al.        | 2005/0205266 A1 | 9/2005 Todd et al.            |  |  |  |  |
| 8,573,295 B2          | 11/2013 Johnson et al.     | 2005/0235757 A1 | 10/2005 De Jonge et al.       |  |  |  |  |
| 8,631,876 B2          | 1/2014 Xu et al.           | 2005/0241824 A1 | 11/2005 Burris, II et al.     |  |  |  |  |
| 8,956,660 B2          | 2/2015 Launag et al.       | 2005/0241825 A1 | 11/2005 Burris, II et al.     |  |  |  |  |
| 9,079,246 B2          | 7/2015 Xu et al.           | 2005/0257936 A1 | 11/2005 Lehr                  |  |  |  |  |
| 9,080,098 B2          | 7/2015 Xu et al.           | 2005/0268746 A1 | 12/2005 Abkowitz et al.       |  |  |  |  |
| 9,260,935 B2          | 2/2016 Murphree et al.     | 2005/0269097 A1 | 12/2005 Towler                |  |  |  |  |
| 2001/0040180 A1       | 11/2001 Wittebrood et al.  | 2005/0275143 A1 | 12/2005 Toth                  |  |  |  |  |
| 2001/0045285 A1       | 11/2001 Russell            | 2005/0279501 A1 | 12/2005 Surjaatmadja et al.   |  |  |  |  |
| 2001/0045288 A1       | 11/2001 Allamon et al.     | 2006/0012087 A1 | 1/2006 Matsuda et al.         |  |  |  |  |
| 2002/0000319 A1       | 1/2002 Brunet              | 2006/0013350 A1 | 1/2006 Akers                  |  |  |  |  |
| 2002/0007948 A1       | 1/2002 Bayne et al.        | 2006/0045787 A1 | 3/2006 Jandeska et al.        |  |  |  |  |
| 2002/0014268 A1       | 2/2002 Vann                | 2006/0057479 A1 | 3/2006 Niimi et al.           |  |  |  |  |
| 2002/0020527 A1       | 2/2002 Kilaas et al.       | 2006/0081378 A1 | 4/2006 Howard et al.          |  |  |  |  |
| 2002/0066572 A1       | 6/2002 Muth                | 2006/0102871 A1 | 5/2006 Wang                   |  |  |  |  |
| 2002/0092654 A1       | 7/2002 Coronado et al.     | 2006/0108114 A1 | 5/2006 Johnson et al.         |  |  |  |  |
| 2002/0096365 A1       | 7/2002 Berscheidt et al.   | 2006/0108126 A1 | 5/2006 Horn et al.            |  |  |  |  |
| 2002/0104616 A1       | 8/2002 De et al.           | 2006/0110615 A1 | 5/2006 Karim et al.           |  |  |  |  |
|                       |                            | 2006/0116696 A1 | 6/2006 Odermatt et al.        |  |  |  |  |
|                       |                            | 2006/0124310 A1 | 6/2006 Lopez De Cerdas et al. |  |  |  |  |
|                       |                            | 2006/0131011 A1 | 6/2006 Lynde et al.           |  |  |  |  |
|                       |                            | 2006/0131031 A1 | 6/2006 McKeachnie et al.      |  |  |  |  |

| (56)                  | References Cited |                          |                 |         |                     |  |  |
|-----------------------|------------------|--------------------------|-----------------|---------|---------------------|--|--|
| U.S. PATENT DOCUMENTS |                  |                          |                 |         |                     |  |  |
| 2006/0131081 A1       | 6/2006           | Mirchandani et al.       | 2008/0196801 A1 | 8/2008  | Zhao et al.         |  |  |
| 2006/0134312 A1       | 6/2006           | Rytlewski et al.         | 2008/0202764 A1 | 8/2008  | Clayton et al.      |  |  |
| 2006/0144515 A1       | 7/2006           | Tada et al.              | 2008/0202814 A1 | 8/2008  | Lyons et al.        |  |  |
| 2006/0150770 A1       | 7/2006           | Freim                    | 2008/0210473 A1 | 9/2008  | Zhang et al.        |  |  |
| 2006/0151178 A1       | 7/2006           | Howard et al.            | 2008/0216383 A1 | 9/2008  | Pierick et al.      |  |  |
| 2006/0153728 A1       | 7/2006           | Schoenung et al.         | 2008/0223586 A1 | 9/2008  | Barnett             |  |  |
| 2006/0162927 A1       | 7/2006           | Walker et al.            | 2008/0223587 A1 | 9/2008  | Cherewyk            |  |  |
| 2006/0169453 A1       | 8/2006           | Savery et al.            | 2008/0236829 A1 | 10/2008 | Lynde               |  |  |
| 2006/0186602 A1       | 8/2006           | Martin et al.            | 2008/0236842 A1 | 10/2008 | Bhavsar et al.      |  |  |
| 2006/0207763 A1       | 9/2006           | Hofman et al.            | 2008/0248205 A1 | 10/2008 | Blanchet et al.     |  |  |
| 2006/0213670 A1       | 9/2006           | Bishop et al.            | 2008/0248413 A1 | 10/2008 | Ishii et al.        |  |  |
| 2006/0231253 A1       | 10/2006          | Vilela et al.            | 2008/0264594 A1 | 10/2008 | Lohmueller et al.   |  |  |
| 2006/0283592 A1       | 12/2006          | Sierra et al.            | 2008/0277109 A1 | 11/2008 | Vaidya              |  |  |
| 2007/0017674 A1       | 1/2007           | Blaisdell                | 2008/0277980 A1 | 11/2008 | Koda et al.         |  |  |
| 2007/0017675 A1       | 1/2007           | Hammami                  | 2008/0282924 A1 | 11/2008 | Saenger et al.      |  |  |
| 2007/0029082 A1       | 2/2007           | Giroux et al.            | 2008/0296024 A1 | 12/2008 | Tianping et al.     |  |  |
| 2007/0039161 A1       | 2/2007           | Garcia                   | 2008/0302538 A1 | 12/2008 | Hofman              |  |  |
| 2007/0039741 A1       | 2/2007           | Hailey                   | 2008/0314581 A1 | 12/2008 | Brown               |  |  |
| 2007/0044958 A1       | 3/2007           | Rytlewski et al.         | 2008/0314588 A1 | 12/2008 | Langlais et al.     |  |  |
| 2007/0044966 A1       | 3/2007           | Davies et al.            | 2009/0038858 A1 | 2/2009  | Griffo et al.       |  |  |
| 2007/0051521 A1       | 3/2007           | Fike et al.              | 2009/0044946 A1 | 2/2009  | Schasteen et al.    |  |  |
| 2007/0053785 A1       | 3/2007           | Hetz et al.              | 2009/0044949 A1 | 2/2009  | King et al.         |  |  |
| 2007/0054101 A1       | 3/2007           | Sigalas et al.           | 2009/0050334 A1 | 2/2009  | Marya et al.        |  |  |
| 2007/0057415 A1       | 3/2007           | Katagiri et al.          | 2009/0056934 A1 | 3/2009  | Xu                  |  |  |
| 2007/0062644 A1       | 3/2007           | Nakamura et al.          | 2009/0065216 A1 | 3/2009  | Frazier             |  |  |
| 2007/0074601 A1       | 4/2007           | Hong et al.              | 2009/0074603 A1 | 3/2009  | Chan et al.         |  |  |
| 2007/0074873 A1       | 4/2007           | McKeachnie et al.        | 2009/0084553 A1 | 4/2009  | Rytlewski et al.    |  |  |
| 2007/0102199 A1       | 5/2007           | Smith et al.             | 2009/0084556 A1 | 4/2009  | Richards et al.     |  |  |
| 2007/0107899 A1       | 5/2007           | Werner et al.            | 2009/0126460 A1 | 4/2009  | Severance           |  |  |
| 2007/0107908 A1       | 5/2007           | Vaidya et al.            | 2009/0090440 A1 | 4/2009  | Kellett et al.      |  |  |
| 2007/0108060 A1       | 5/2007           | Park                     | 2009/0107684 A1 | 4/2009  | Cooke, Jr.          |  |  |
| 2007/0119600 A1       | 5/2007           | Slup et al.              | 2009/0114381 A1 | 5/2009  | Stroobants          |  |  |
| 2007/0131912 A1       | 6/2007           | Simone et al.            | 2009/0114382 A1 | 5/2009  | Grove et al.        |  |  |
| 2007/0151009 A1       | 7/2007           | Conrad, III et al.       | 2009/0126436 A1 | 5/2009  | Fly et al.          |  |  |
| 2007/0151769 A1       | 7/2007           | Slutz et al.             | 2009/0139720 A1 | 6/2009  | Frazier             |  |  |
| 2007/0169935 A1       | 7/2007           | Akbar et al.             | 2009/0145666 A1 | 6/2009  | Radford et al.      |  |  |
| 2007/0181224 A1       | 8/2007           | Marya et al.             | 2009/0151949 A1 | 6/2009  | Marya et al.        |  |  |
| 2007/0185655 A1       | 8/2007           | Le Bemadjiel             | 2009/0152009 A1 | 6/2009  | Slay et al.         |  |  |
| 2007/0187095 A1       | 8/2007           | Walker et al.            | 2009/0155616 A1 | 6/2009  | Thamida et al.      |  |  |
| 2007/0207182 A1       | 9/2007           | Weber et al.             | 2009/0159289 A1 | 6/2009  | Avant et al.        |  |  |
| 2007/0221373 A1       | 9/2007           | Murray                   | 2009/0178808 A1 | 7/2009  | Williamson et al.   |  |  |
| 2007/0221384 A1       | 9/2007           | Murray                   | 2009/0194273 A1 | 8/2009  | Surjaatmadja et al. |  |  |
| 2007/0227745 A1       | 10/2007          | Roberts et al.           | 2009/0205841 A1 | 8/2009  | Kluge et al.        |  |  |
| 2007/0259994 A1       | 11/2007          | Tour et al.              | 2009/0211770 A1 | 8/2009  | Nutley et al.       |  |  |
| 2007/0261862 A1       | 11/2007          | Murray                   | 2009/0226340 A1 | 9/2009  | Marya               |  |  |
| 2007/0272411 A1       | 11/2007          | Lopez De Cardenas et al. | 2009/0226704 A1 | 9/2009  | Kauppinen et al.    |  |  |
| 2007/0272413 A1       | 11/2007          | Rytlewski et al.         | 2009/0242202 A1 | 10/2009 | Rispler et al.      |  |  |
| 2007/0277979 A1       | 12/2007          | Todd et al.              | 2009/0242208 A1 | 10/2009 | Bolding             |  |  |
| 2007/0284109 A1       | 12/2007          | East et al.              | 2009/0242214 A1 | 10/2009 | Foster et al.       |  |  |
| 2007/0284112 A1       | 12/2007          | Magne et al.             | 2009/0255667 A1 | 10/2009 | Clem et al.         |  |  |
| 2007/0299510 A1       | 12/2007          | Venkatraman et al.       | 2009/0255684 A1 | 10/2009 | Bolding             |  |  |
| 2008/0011473 A1       | 1/2008           | Wood et al.              | 2009/0255686 A1 | 10/2009 | Richard             |  |  |
| 2008/0020923 A1       | 1/2008           | Debe et al.              | 2009/0266548 A1 | 10/2009 | Olsen et al.        |  |  |
| 2008/0047707 A1       | 2/2008           | Boney et al.             | 2009/0260817 A1 | 11/2009 | Gambier et al.      |  |  |
| 2008/0060810 A9       | 3/2008           | Nguyen et al.            | 2009/0272544 A1 | 11/2009 | Giroux et al.       |  |  |
| 2008/0066923 A1       | 3/2008           | Xu                       | 2009/0283270 A1 | 11/2009 | Langeslag           |  |  |
| 2008/0066924 A1       | 3/2008           | Xu                       | 2009/0293672 A1 | 12/2009 | Mirchandani et al.  |  |  |
| 2008/0072705 A1       | 3/2008           | Chaumonnot et al.        | 2009/0301730 A1 | 12/2009 | Gweily              |  |  |
| 2008/0078553 A1       | 4/2008           | George                   | 2009/0305131 A1 | 12/2009 | Kumar et al.        |  |  |
| 2008/0081866 A1       | 4/2008           | Gong et al.              | 2009/0308588 A1 | 12/2009 | Howell et al.       |  |  |
| 2008/0093073 A1       | 4/2008           | Bustos et al.            | 2009/0317556 A1 | 12/2009 | Macary              |  |  |
| 2008/0099209 A1       | 5/2008           | Loretz et al.            | 2009/0317622 A1 | 12/2009 | Huang et al.        |  |  |
| 2008/0105438 A1       | 5/2008           | Jordan et al.            | 2010/0003536 A1 | 1/2010  | Smith et al.        |  |  |
| 2008/0115932 A1       | 5/2008           | Cooke                    | 2010/0012385 A1 | 1/2010  | Drivdahl et al.     |  |  |
| 2008/0121390 A1       | 5/2008           | O'Malley et al.          | 2010/0015002 A1 | 1/2010  | Barrera et al.      |  |  |
| 2008/0121436 A1       | 5/2008           | Slay et al.              | 2010/0015469 A1 | 1/2010  | Romanowski et al.   |  |  |
| 2008/0127475 A1       | 6/2008           | Griffo                   | 2010/0025255 A1 | 2/2010  | Su et al.           |  |  |
| 2008/0135249 A1       | 6/2008           | Fripp et al.             | 2010/0032151 A1 | 2/2010  | Duphorne et al.     |  |  |
| 2008/0149325 A1       | 6/2008           | Crawford                 | 2010/0034857 A1 | 2/2010  | Launag et al.       |  |  |
| 2008/0149345 A1       | 6/2008           | Bicerano                 | 2010/0038076 A1 | 2/2010  | Spray et al.        |  |  |
| 2008/0149351 A1       | 6/2008           | Marya et al.             | 2010/0038595 A1 | 2/2010  | Imholt et al.       |  |  |
| 2008/0169105 A1       | 7/2008           | Williamson et al.        | 2010/0040180 A1 | 2/2010  | Kim et al.          |  |  |
| 2008/0169130 A1       | 7/2008           | Norman et al.            | 2010/0044041 A1 | 2/2010  | Smith et al.        |  |  |
| 2008/0179060 A1       | 7/2008           | Surjaatmadja et al.      | 2010/0051278 A1 | 3/2010  | Mytopher et al.     |  |  |
| 2008/0179104 A1       | 7/2008           | Zhang et al.             | 2010/0055491 A1 | 3/2010  | Vecchio et al.      |  |  |
|                       |                  |                          | 2010/0055492 A1 | 3/2010  | Barsoum et al.      |  |  |
|                       |                  |                          | 2010/0089583 A1 | 4/2010  | Xu et al.           |  |  |
|                       |                  |                          | 2010/0089587 A1 | 4/2010  | Stout               |  |  |
|                       |                  |                          | 2010/0101803 A1 | 4/2010  | Clayton et al.      |  |  |

| (56)                  | References Cited |                          |                 |         |                  |         |
|-----------------------|------------------|--------------------------|-----------------|---------|------------------|---------|
| U.S. PATENT DOCUMENTS |                  |                          |                 |         |                  |         |
| 2010/0116495 A1       | 5/2010           | Spray                    | 2012/0292053 A1 | 11/2012 | Xu et al.        |         |
| 2010/0122817 A1       | 5/2010           | Surjaatmadja et al.      | 2012/0318513 A1 | 12/2012 | Mazyar et al.    |         |
| 2010/0139930 A1       | 6/2010           | Patel et al.             | 2013/0004847 A1 | 1/2013  | Kumar et al.     |         |
| 2010/0200230 A1       | 8/2010           | East, Jr. et al.         | 2013/0008671 A1 | 1/2013  | Booth et al.     |         |
| 2010/0236793 A1       | 9/2010           | Bjorgum                  | 2013/0025409 A1 | 1/2013  | Xu               |         |
| 2010/0236794 A1       | 9/2010           | Duan et al.              | 2013/0029886 A1 | 1/2013  | Mazyar et al.    |         |
| 2010/0243254 A1       | 9/2010           | Murphy et al.            | 2013/0032357 A1 | 2/2013  | Mazyar et al.    |         |
| 2010/0252273 A1       | 10/2010          | Duphorne                 | 2013/0048304 A1 | 2/2013  | Agrawal et al.   |         |
| 2010/0252280 A1       | 10/2010          | Swor et al.              | 2013/0048305 A1 | 2/2013  | Xu et al.        |         |
| 2010/0270031 A1       | 10/2010          | Patel                    | 2013/0052472 A1 | 2/2013  | Xu               |         |
| 2010/0276136 A1       | 11/2010          | Evans et al.             | 2013/0081814 A1 | 4/2013  | Gaudette et al.  |         |
| 2010/0276159 A1       | 11/2010          | Mailand et al.           | 2013/0084643 A1 | 4/2013  | Commarieu et al. |         |
| 2010/0282338 A1       | 11/2010          | Gerrard et al.           | 2013/0105159 A1 | 5/2013  | Alvarez          |         |
| 2010/0282469 A1       | 11/2010          | Richard et al.           | 2013/0126190 A1 | 5/2013  | Mazyar et al.    |         |
| 2010/0294510 A1       | 11/2010          | Holmes                   | 2013/0133897 A1 | 5/2013  | Baihly et al.    |         |
| 2010/0297432 A1       | 11/2010          | Sherman et al.           | 2013/0146144 A1 | 6/2013  | Joseph et al.    |         |
| 2010/0304182 A1       | 12/2010          | Facchini et al.          | 2013/0146302 A1 | 6/2013  | Gaudette et al.  |         |
| 2010/0314105 A1       | 12/2010          | Rose                     | 2013/0168257 A1 | 7/2013  | Mazyar et al.    |         |
| 2010/0314126 A1*      | 12/2010          | Kellner .....            | 2013/0186626 A1 | 7/2013  | Aitken et al.    |         |
|                       |                  | E21B 34/14               | 2013/0240200 A1 | 9/2013  | Frazier          |         |
|                       |                  | 166/373                  | 2013/0240203 A1 | 9/2013  | Frazier          |         |
| 2010/0319870 A1       | 12/2010          | Bewlay et al.            | 2013/0299185 A1 | 11/2013 | Xu et al.        |         |
| 2010/0326650 A1       | 12/2010          | Tran et al.              | 2013/0299192 A1 | 11/2013 | Xu et al.        |         |
| 2011/0005773 A1       | 1/2011           | Dusterhoff et al.        | 2013/0300066 A1 | 11/2013 | Xu et al.        |         |
| 2011/0036592 A1       | 2/2011           | Fay                      | 2013/0319668 A1 | 12/2013 | Tschetter et al. |         |
| 2011/0048743 A1       | 3/2011           | Stafford et al.          | 2013/0327540 A1 | 12/2013 | Hamid et al.     |         |
| 2011/0052805 A1       | 3/2011           | Bordere et al.           | 2014/0014339 A1 | 1/2014  | O'Malley et al.  |         |
| 2011/0056692 A1       | 3/2011           | Lopez De Cardenas et al. | 2014/0027128 A1 | 1/2014  | Johnson et al.   |         |
| 2011/0056702 A1       | 3/2011           | Sharma et al.            | 2014/0060834 A1 | 3/2014  | Quintero et al.  |         |
| 2011/0067872 A1       | 3/2011           | Agrawal                  | 2014/0116711 A1 | 5/2014  | Tang et al.      |         |
| 2011/0067889 A1       | 3/2011           | Marya et al.             | 2014/0262327 A1 | 9/2014  | Xu et al.        |         |
| 2011/0067890 A1       | 3/2011           | Themig                   | 2014/0360728 A1 | 12/2014 | Tashiro et al.   |         |
| 2011/0094406 A1       | 4/2011           | Marya et al.             | 2015/0060085 A1 | 3/2015  | Xu               |         |
| 2011/0100643 A1       | 5/2011           | Themig et al.            | 2015/0065401 A1 | 3/2015  | Xu et al.        |         |
| 2011/0127044 A1       | 6/2011           | Radford et al.           | 2016/0209391 A1 | 7/2016  | Zhang et al.     |         |
| 2011/0132143 A1       | 6/2011           | Xu et al.                | 2016/0258242 A1 | 9/2016  | Hayter et al.    |         |
| 2011/0132612 A1       | 6/2011           | Agrawal et al.           |                 |         |                  |         |
| 2011/0132619 A1*      | 6/2011           | Agrawal .....            | E21B 23/04      | CN      | 1076968 A        | 10/1993 |
|                       |                  | 166/376                  |                 | CN      | 1079234 A        | 12/1993 |
| 2011/0132620 A1       | 6/2011           | Agrawal et al.           |                 | CN      | 1255879 A        | 6/2000  |
| 2011/0132621 A1       | 6/2011           | Agrawal et al.           |                 | CN      | 2658384 Y        | 11/2004 |
| 2011/0135530 A1       | 6/2011           | Xu et al.                |                 | CN      | 1668545 A        | 9/2005  |
| 2011/0135805 A1       | 6/2011           | Doucet et al.            |                 | CN      | 101050417 A      | 10/2007 |
| 2011/0135953 A1       | 6/2011           | Xu et al.                |                 | CN      | 101351523 A      | 1/2009  |
| 2011/0136707 A1       | 6/2011           | Xu et al.                |                 | CN      | 101454074 A      | 6/2009  |
| 2011/0139465 A1       | 6/2011           | Tibbles et al.           |                 | CN      | 101457321 A      | 6/2009  |
| 2011/0147014 A1       | 6/2011           | Chen et al.              |                 | CN      | 101605963        | 12/2009 |
| 2011/0186306 A1       | 8/2011           | Marya et al.             |                 | CN      | 101720378 A      | 6/2010  |
| 2011/0214881 A1       | 9/2011           | Newton                   |                 | EP      | 0033625 A1       | 8/1981  |
| 2011/0247833 A1       | 10/2011          | Todd et al.              |                 | EP      | 1174385 A2       | 1/2002  |
| 2011/0253387 A1       | 10/2011          | Ervin                    |                 | EP      | 1412175 A1       | 4/2004  |
| 2011/0256356 A1       | 10/2011          | Tomantschger et al.      |                 | EP      | 1798301 A1       | 8/2006  |
| 2011/0259610 A1       | 10/2011          | Shkurti et al.           |                 | EP      | 1857570 A2       | 11/2007 |
| 2011/0277987 A1       | 11/2011          | Frazier                  |                 | FR      | 2782096 A1       | 2/2000  |
| 2011/0277989 A1       | 11/2011          | Frazier                  |                 | GB      | 912956 A         | 12/1962 |
| 2011/0284232 A1       | 11/2011          | Huang                    |                 | GB      | 1046330 A        | 10/1966 |
| 2011/0284240 A1       | 11/2011          | Chen et al.              |                 | GB      | 1280833 A        | 7/1972  |
| 2011/0284243 A1       | 11/2011          | Frazier                  |                 | GB      | 1357065 A        | 6/1974  |
| 2011/0300403 A1       | 12/2011          | Vecchio et al.           |                 | JP      | 61067770 A       | 4/1986  |
| 2011/0314881 A1       | 12/2011          | Hatcher et al.           |                 | JP      | 754008 A         | 2/1995  |
| 2012/0067426 A1       | 3/2012           | Soni et al.              |                 | JP      | 8232029 A        | 9/1996  |
| 2012/0090839 A1       | 4/2012           | Rudic                    |                 | JP      | 2000185725 A1    | 7/2000  |
| 2012/0103135 A1       | 5/2012           | Xu et al.                |                 | JP      | 2002053902 A     | 2/2002  |
| 2012/0107590 A1       | 5/2012           | Xu et al.                |                 | JP      | 2004225084 A     | 8/2004  |
| 2012/0118583 A1       | 5/2012           | Johnson et al.           |                 | JP      | 2004225765 A     | 8/2004  |
| 2012/0130470 A1       | 5/2012           | Agnew                    |                 | JP      | 2005076052 A     | 3/2005  |
| 2012/0145378 A1       | 6/2012           | Frazier et al.           |                 | JP      | 2010502840 A     | 1/2010  |
| 2012/0145389 A1       | 6/2012           | Fitzpatrick, Jr.         |                 | KR      | 950014350 B1     | 11/1995 |
| 2012/0168152 A1       | 7/2012           | Casciaro et al.          |                 | WO      | 9909227 A1       | 2/1999  |
| 2012/0177905 A1       | 7/2012           | Seals et al.             |                 | WO      | 9947726 A1       | 9/1999  |
| 2012/0205120 A1       | 8/2012           | Howell                   |                 | WO      | 2004001087 A1    | 12/2003 |
| 2012/0205872 A1       | 8/2012           | Reinhardt et al.         |                 | WO      | 2004073889 A1    | 9/2004  |
| 2012/0211239 A1       | 8/2012           | Kritzler et al.          |                 | WO      | 2005040068 A     | 5/2005  |
| 2012/0234546 A1       | 9/2012           | Xu et al.                |                 | WO      | 2007044635 A     | 4/2007  |
| 2012/0234547 A1       | 9/2012           | O'Malley et al.          |                 | WO      | 2007095376 A2    | 8/2007  |
| 2012/0267101 A1       | 10/2012          | Cooke                    |                 | WO      | 2008034042 A3    | 3/2008  |
|                       |                  |                          |                 | WO      | 2008057045 A1    | 5/2008  |

## FOREIGN PATENT DOCUMENTS

(56)

## References Cited

## FOREIGN PATENT DOCUMENTS

|    |            |    |         |
|----|------------|----|---------|
| WO | 2008079485 | A2 | 7/2008  |
| WO | 2008079777 | A2 | 7/2008  |
| WO | 2009079745 | A1 | 7/2009  |
| WO | 2010012184 | A1 | 2/2010  |
| WO | 2011071902 | A2 | 6/2011  |
| WO | 2011071907 | A2 | 6/2011  |
| WO | 2011071910 | A2 | 6/2011  |
| WO | 2011130063 | A3 | 2/2012  |
| WO | 2012015567 | A2 | 2/2012  |
| WO | 2012149007 | A2 | 11/2012 |
| WO | 2012174101 | A2 | 12/2012 |
| WO | 2013053057 | A1 | 4/2013  |
| WO | 2013078031 | A1 | 5/2013  |
| WO | 2014121384 | A1 | 8/2014  |

## OTHER PUBLICATIONS

- Aviles et al, "Degradable Alternative to Risky Mill-Out Operations in Plug and Perf"; SPE-173695-MS; Society of Petroleum Engineers; SPE/ICOTA Coiled Tubing & Well Intervention Conference & Exhibition; March 24-25, 2015; 10 pages.
- Ayman, et al.; "Effect of Consolidation and Extrusion Temperatures on Tensile Properties of Hot Extruded ZK61 Magnesium Alloy Gas Atomized Powders via Spark Plasma Sintering", Transactions of JWRI, vol. 38 (2009), No. 2, pp. 1-5.
- Baker Hughes Incorporated. IN-Tallie Disintegrating Frac Balls. Houston: Baker Hughes Incorporated, 2011. Accessed Mar. 6, 2015.
- Baker Hughes, "Multistage", Oct. 31, 2011, BakerHughes.com; accessed Mar. 6, 2015.
- Bin et al., "Advances in Fluidization CVD Technology", East China University of Chemical Technology, China Academic Journal Electronic Publishing House, vol. 13, No. 4, Nov. 1992, pp. 360-365, English Abstract on p. 366.
- Chuan-Jun et al., "Study on Corrosion Kinetics of Mg-Ni alloys", Journal of Kunming University of Science and Technology, vol. 34, No. 5, pp. 10-13, Oct. 2009.
- International Search Report and Written Opinion, International Application No. PCT/US2016/041849, dated Oct. 26, 2016, Korean Intellectual Property Office; International Search Report 5 pages, Written Opinion 7 pages.
- Lin et al., "Processing and Microstructure of Nano-Mo/Al<sub>2</sub>O<sub>3</sub> Composites from MOCVD and Fluidized Bed", Nanostructured Materials, Nov. 1999, vol. 11, No. 8, pp. 1361-1377.
- M.S. Senthil Saravanan et al, "Mechanically Alloyed Carbon Nanotubes (CNT) Reinforced Nanocrystalline AA 4032: Synthesis and Characterization", Journal of Minerals and Materials Characterization and Engineering, vol. 9, No. 11 pp. 1027-1035 2010.
- Reid, Gary Carl, "Literature evaluation of induced groundwater tracers, field tracer techniques, and hydrodynamic dispersion values in porous media", Thesis in Geosciences (Masters), Texas Tech University, Aug. 1981, 109 pages.
- Rose, et al.; "The application of the polyaromatic sulfonates as tracers in geothermal reservoirs", Geothermics 30 (2001) pp. 617-640.
- Shigematsu, et al., "Surface Treatment of AZ91D Magnesium Alloy by Aluminum diffusion Coating", Journal of Materials Science Letters 19, 2000, pp. 473-475.
- Singh, et al., "Extended Homogeneity Range of Intermetallic Phases in Mechanically Alloyed Mg-Al Alloys", Elsevier Sciences Ltd., Intemetallics 11, 2003, pp. 373-376.
- Spencer et al., "Fluidized Bed Polymer Particle ALD Process for Producing HDPE/Alumina Nanocomposites", The 12th International Conference on Fluidization—New Horizons in Fluidization Engineering, vol. RP4 (2007).
- Stanley, et al.; "An Introduction to Ground-Water Tracers", Department of Hydrology and Water Resources, University of Arizona, Mar. 1985, pp. 1-219.
- Tsipas et al. "Effect of High Energy Ball Milling on Titanium-Hydroxyapatite Powders" Powder Metallurgy, Maney Publishing, London, GB, vol. 46, No. 1, Mar. 2003 (Mar. 2003), pp. 73-77.
- Zemel, "Tracers in the Oil Field", University of Texas at Austin, Center for Petroleum and Geosystems, Jan. 1995, Chapters 1, 2, 3, 7.
- "Baker Hughes Refines Expandable Tubular Technology with Abaqus and Isight", Simulia Realistic Simulation News, Jan./Feb. 2011, pp. 12-13.
- "Reactivity series", Wikipedia, [http://en.wikipedia.org/w/index.php?title=Reactivity\\_series&printable=yes](http://en.wikipedia.org/w/index.php?title=Reactivity_series&printable=yes) downloaded on May 18, 2014. 8 pages.
- Bakshi et al., "Carbon nanotube reinforced metal matrix composites—a review," International Materials Reviews; 2010, pp. 41-64, vol. 55, No. 1.
- Birbilis, et al., "Exploring Corrosion Protection of Mg Via Ionic Liquid Pretreatment", Surface & Coatings Technology; 201, pp. 4496-4504, (2007).
- Feng, et al., "Electroless Plating of Carbon Nanotubes with Silver" Journal of Materials Science, 39, (2004) pp. 3241-3243.
- Lee, et al., "Effects of Ni addition on hydrogen storage properties of Mg17Al12 alloy", Materials Chemistry and Physics, 2011, 126, pp. 319-324.
- Li, et al., "Investigation of aluminium-based nanocomposites with ultra-high strength", Materials Science and Engineering A, 527, pp. 305-316, (2009).
- Liu, et al.; "Electroless Nickel Plating on AZ91 Mg Alloy Substrate"; Surface & Coatings Technology; 200, pp. 5087-5093; (2006).
- Mathis, "Sand Management: A Review of Approaches and Concerns", Society of Petroleum Engineers, SPE Paper No. 82240, SPE European Formation Damage Conference, The Hague, The Netherlands, May 13-14, 2003.
- Pardo, et al.; "Corrosion Behaviour of Magnesium/Aluminium Alloys in 3.5 wt% NaCl"; Corrosion Science; 50; pp. 823-834; (2008).
- Quik Drill Composite Frac Plug; Baker Hughes, Baker Oil Tools; Copyright 2002; 3 pages.
- Shi, et al.; "Influence of the Beta Phase on the Corrosion Performance of Anodised Coatings on Magnesium-Aluminium Alloys"; Corrosion Science; 47; pp. 2760-2777; (2005).
- Shimizu, et al., "Multi-walled carbon nanotube-reinforced magnesium alloy composites", Scripta Materialia, vol. 58, Issue 4, Feb. 2008, pp. 267-270.
- Shumbera, et al. "Improved Water Injector Performance in a Gulf of Mexico Deepwater Development Using an Openhole Frac Pack Completion and Downhole Filter System: Case History." SPE Annual Technical Conference and Exhibition, Oct. 5-8, 2003.
- Song, et al.; "Corrosion Mechanisms of Magnesium Alloys"; Advanced Engineering Materials; 1(1); pp. 11-33; (1999).
- Song, et al.; "Influence of Microstructure on the Corrosion of Diecast AZ91D"; Corrosion Science; 41; pp. 249-273; (1999).
- Song, et al.; "Understanding Magnesium Corrosion"; Advanced Engineering Materials; 5; No. 12; pp. 837-858; (2003).
- Sun, et al.; "Colloidal Processing of Carbon Nanotube/Alumina Composites" Chem. Mater. 2002, 14, pp. 5169-5172.
- Vickery, et al.; "New One-Trip Multi-Zone Frac Pack System with Positive Positioning." European Petroleum Conference, Oct. 29-31, 2002, Aberdeen, UK. [Abstract Only].
- Zeng, et al. "Progress and Challenge for Magnesium Alloys as Biomaterials," Advanced Engineering Materials, vol. 10, Issue 8, Aug. 2008, pp. B3-B14.
- Zhang, et al.; "High Strength Nanostructured Materials and Their Oil Field Applications", Society of Petroleum Engineers; Conference Paper SPE 157092; SPE International Oilfield Nanotechnology Conference, 2012; 6 pages.
- Zhang, et al.; "Metal Coating on Suspended Carbon Nanotubes and its Implication to Metal-Tube Interaction", Chemical Physics Letters 331 (2000) 35-41.
- "Optisleeve Sliding Sleeve", [online]; [retrieved on Jun. 25, 2010]; retrieved from the Internet [weatherfordcorp/WFT033159.pdf](http://weatherford.com/weatherford/groups/.../weatherfordcorp/WFT033159.pdf).

(56)

## References Cited

## OTHER PUBLICATIONS

- Baker Hughes, "Flow Control Systems," [online]; [retrieved on May 20, 2010]; retrieved from the Internet <http://www.bakerhughes.com/products-and-services/completions-and-productions/well-completions/packers-and-flow-control/flow-control-systems>.
- Bououdina, et al., "Comparative Study of Mechanical Alloying of (Mg+Al) and (Mg+Al+Ni) Mixtures for Hydrogen Storage", *J. Alloys. Compds.* 2002, 336, 222-231.
- Carrejo, et al., "Improving Flow Assurance in Multi-Zone Fracturing Treatments in Hydrocarbon Reservoirs with High Strength Coorable Tripping Balls"; Society of Petroleum Engineers; SPE Paper No. 151613; Apr. 16, 2012; 6 pages.
- Coronado, "Development of an Internal Coiled Tubing Connector Utilizing Permanent Packer Technology"; Society of Petroleum Engineers, SPE Paper No. 46036; Apr. 15, 1998; 10 pages.
- Garfield, New One-Trip Sand-Control Completion System that Eliminates Formation Damage Resulting From conventional Perforating and Gravel-Pack Operations;, SPE Annual Technical Conference and Exhibition, Oct. 9-12, 2005.
- Gray, et al., "Protective Coatings on Magnesium and Its Alloys—a Critical Review", *Journal of Alloys and Compounds* 336 (2002), pp. 88-113.
- Hsiao, et al., "Anodization of AZ91D Magnesium Alloy in Silicate-Containing Electrolytes"; *Surface & Coatings Technology*; 199; pp. 127-134; (2005).
- Hsiao, et al., "Characterization of Anodic Films Formed on AZ91D Magnesium Alloy"; *Surface & Coatings Technology*; 190; pp. 299-308; (2005).
- Huo et al.; "Corrosion of AZ91D Magnesium Alloy with a Chemical Conversion Coating and Electroless Nickel Layer"; *Corrosion Science*; 46; pp. 1467-1477; (2004).
- Kuzumaki, et al.; "Mechanical Characteristics and Preparation of Carbon Nanotube Fiber-Reinforced Ti Composite", *Advanced Engineering Materials*, 2000, 2, No. 7.
- Liu, et al., "Calculated Phase Diagrams and the Corrosion of Die-Cast Mg-Al Alloys", *Corrosion Science*, 2009, 51, 606-619.
- Lunder et al.; "The Role of Mg17Al12 Phase in the Corrosion of Mg Alloy AZ91"; *Corrosion*; 45(9); pp. 741-748; (1989).
- Majumdar, et al., "Laser Surface Engineering of a Magnesium Alloy with Al + Al2O3", *Surface and Coatings Technology* 179 (2004) pp. 297-305.
- Murray, "Binary Alloy Phase Diagrams" *Int. Met. Rev.*, 30(5) 1985 vol. 1, pp. 103-187.
- Nie, "Patents of Methods to Prepare Intermetallic Matrix Composites: A Review", *Recent Patents on Materials Science* 2008, vol. 1, pp. 232-240.
- Saravanan et al., "Mechanically Alloyed Carbon Nanotubes (CNT) Reinforced Nanocrystalline AA 4032: Synthesis and Characterization," *Journal of Minerals & Materials Characterization & Engineering*, vol. 9, No. 11, pp. 1027-1035, 2010.
- Shaw, "Benefits and Application of a Surface-Controlled Sliding Sleeve for Fracturing Operations"; Society of Petroleum Engineers, SPE Paper No. 147546; Oct. 30, 2011; 8 pages.
- Song, "Recent Progress in Corrosion and Protection of Magnesium Alloys"; *Advanced Engineering Materials*; 7(7); pp. 563-586; (2005).
- Song, et al.; "A Possible Biodegradable Magnesium Implant Material," *Advanced Engineering Materials*, vol. 9, Issue 4, Apr. 2007, pp. 298-302.
- Song, et al.; "Corrosion Behaviour of AZ21, AZ501 and AZ91 in Sodium Chloride"; *Corrosion Science*; 40(10); pp. 1769-1791; (1998).
- Triolo et al., "Resolving the Completion Engineer's Dilemma: Permanent or Retrievable Packer?"; Society of Petroleum Engineers, SPE Paper No. 76711; May 20, 2002; 16 pages.
- Vernon Constien et al., "Development of Reactive Coatings to Protect Sand-Control Screens", SPE 112494, Copyright 2008, Society of Petroleum Engineers, Presented at the 2008 SPE International Symposium and Exhibition on Formation Damage Control.
- Walters, et al.; "A Study of Jets from Unsintered-Powder Metal Lined Nonprecision Small-Caliber Shaped Charges", Army Research Laboratory, Aberdeen Proving Ground, MD 21005-5066; Feb. 2001.
- Wang, et al., "Contact-Damage-Resistant Ceramic/Single-Wall Carbon Nanotubes and Ceramic/Graphite Composites" *Nature Materials*, vol. 3, Aug. 2004, pp. 539-544.
- Watanabe, et al., "Superplastic Deformation Mechanism in Powder Metallurgy Magnesium Alloys and Composites", *Acta mater.* 49 (2001) pp. 2027-2037.
- Watarai, Trend of research and development for magnesium alloys-reducing the weight of structural materials in motor vehicles, (2006) *Science and technology trends, Quaterly review* No. 18, 84-97.
- Welch, et al., "Nonelastomeric Sliding Sleeve Maintains Long Term Integrity in HP/HT Application: Case Histories" [Abstract Only], SPE Eastern Regional Meeting, Oct. 23-25, 1996, Columbus. Ohio.
- Xu, et al., "Nanostructured Material-Based Completion Tools Enhance Well Productivity"; *International Petroleum Technology Conference*; Conference Paper IPTC 16538; *International Petroleum Technology Conference* 2013; 4 pages.
- Zhan, et al., "Single-wall carbon nanotubes as attractive toughening agents in alumina-based nanocomposites" *Nature Materials*, vol. 2., Jan. 2003, pp. 38-42.
- Zhang, et al.; "Formation of metal nanowires on suspended single-walled carbon nanotubes" *Applied Physics Letter*, vol. 77, No. 19 (2000), pp. 3015-3017.
- Zhang, et al.; "Study on the Environmentally Friendly Anodizing of AZ91D Magnesium Alloy"; *Surface and Coatings Technology*: 161; pp. 36-43; (2002).
- Zhu, et al., "The process of coating on ultrafine particles by surface hydrolysis reaction in a fluidized bed reactor", *Surface and Coatings Technology* 135 (2000) 14-17.
- "Sliding Sleeve", Omega Completion Technology Ltd, Sep. 29, 2009, retrieved on: [www.omega-completion.com](http://www.omega-completion.com).
- Ambat, et al., "Electroless Nickel-Plating on AZ91D Magnesium Alloy: Effect of Substrate Microstructure and Plating Parameters"; *Surface and Coatings Technology*; 179; pp. 124-134; (2004).
- Baker Oil Tools, "Baker Oil Tools Introduces Revolutionary Sand Control Completion Technology," May 2, 2005.
- Baker Oil Tools, "Z-Seal Metal-to-Metal Expandable Sealing Device Uses Expanding Metal in Place of Elastomers," Nov. 6, 2006.
- Bastow, et al., "Clustering and formation of nano-precipitates in dilute aluminum and magnesium alloys", *Materials Science and Engineering*, 2003, C23, 757-762.
- Bercegeay, et al., "A One-Trip Gravel Packing System"; Society of Petroleum Engineers, Offshore Technology Conference, SPE Paper No. 4771; Feb. 7-8, 1974.
- Bybee, "One-Trip Completion System Eliminates Perforations," *Completions Today*, Sep. 2007, pp. 52-53.
- Chang, et al., "Electrodeposition of Aluminum on Magnesium Alloy in Aluminum Chloride (AlCl3)-1-ethyl-3-methylimidazolium chloride (EMIC) Ionic Liquid and Its Corrosion Behavior"; *Electrochemistry Communications*; 9; pp. 1602-1606; (2007).
- Christoglou, et al., "Deposition of Aluminum on Magnesium by a CVD Process", *Surface and Coatings Technology* 184 (2004) 149-155.
- Constantine, "Selective Production of Horizontal Openhole Completions Using ECP and Sliding Sleeve Technology." *SPE Rocky Mountain Regional Meeting*, May 15-18, 1999, Gillette, Wyoming. [Abstract Only].
- Curtin, et al., "CNT-reinforced ceramics and metals," *Materials Today*, 2004, vol. 7, pp. 44-49.
- Flahaut, et al., "Carbon Nanotube-Metal-Oxide Nanocomposites: Microstructure, Electrical Conductivity and Mechanical Properties" *Acta mater.* 48 (2000), pp. 3803-3812.
- Forsyth, et al.; "An Ionic Liquid Surface Treatment for Corrosion Protection of Magnesium Alloy AZ31"; *Electrochim. Solid-State Lett.* 2006 vol. 9, Issue 11, B52-B55/ 9(11); ABSTRACT only; 1 page.
- Galanty, et al. "Consolidation of metal powders during the extrusion process," *Journal of Materials Processing Technology* (2002), pp. 491-496.

(56)

**References Cited****OTHER PUBLICATIONS**

- Garfield, "Formation Damage Control Utilizing Composite-Bridge-Plug Technology for Monobore, Multizone Stimulation Operations," SPE 70004, 2001, Society of Petroleum Engineers Inc., This paper was prepared for presentation at the SPE Per.
- Garfield, et al., "Maximizing Inflow Performance in Soft Sand Completions Using New One-trip Sand Control Liner Completion Technology", SPE European Formation Damage Conference, May 25-27, 2005.
- Goh, et al., "Development of novel carbon nanotube reinforced magnesium nanocomposites using the powder metallurgy technique", Nanotechnology 17 (2006) 7-12.
- Han, et al., "Mechanical Properties of Nanostructured Materials", Rev. Adv. Mater. Sci. 9(2005) 1-16.
- Hermawan, et al., "Iron-manganese: new class of metallic degradable biomaterials prepared by powder metallurgy", Powder Metallurgy, vol. 51, No. 1, (2008), pp. 38-45.
- Hjortstam, et al. "Can we achieve ultra-low resistivity in carbon nanotube-based metal composites," Applied Physics A (2004), vol. 78, Issue 8, pp. 1175-1179.
- Hsiao, et al., "Baking Treatment Effect on Materials Characteristics and Electrochemical Behavior of anodic Film Formed on AZ91D Magnesium Alloy"; Corrosion Science; 49; pp. 781-793; (2007).
- Hsiao, et al., "Effect of Heat Treatment on Anodization and Electrochemical Behavior of AZ91D Magnesium Alloy"; J. Mater. Res.; 20(10); pp. 2763-2771;(2005).
- Lavernia, et al.. "Cryomilled Nanostructured Materials: Processing and Properties", Materials Science and Engineering A, 493, (2008) pp. 207-214.
- Li, "Design of Abrasive Water Jet Perforation and Hydraulic Fracturing Tool," Oil Field Equipment, Mar. 2011.
- Maisano, "Cryomilling of Aluminum-Based and Magnesium-Based Metal Powders", Thesis, Virginia Tech, Jan. 13, 2006.
- Seyni, et al., "On the interest of using degradable fillers in co-ground composite materials", Powder Technology 190, (2009) pp. 176-184.
- Vahlas, et al., "Principles and Applications of CVD Powder Technology", Materials Science and Engineering R 53 (2006) pp. 1-72.
- Australian Examination Report, Australian Application No. 2012271765, dated Feb. 28, 2017, Australian Intellectual Property Office; Australian Examination Report 3 pages.
- "Declaration of Karl T. Hartwig in Support of Petitioner Pursuant to 37 C.F.R. § 42.120", executed on Nov. 21, 2016 in support of U.S. Pat. No. 8,573,295, 52 pages.
- "Declaration of Karl T. Hartwig in Support of Petitioner Pursuant to 37 C.F.R. § 42.120", executed on Nov. 21, 2016 in support of U.S. Pat. No. 9,101,978, 51 pages.
- Callister, Jr., William D., Materials Science and Engineering An Introduction, Seventh Edition, 2006, pp. 111, 627, and G7.
- German, Randall M., Powder Metallurgy Science, Second Edition, 1994, 102 pages.
- Klar, Erhard, ASM Handbook: International Metals Handbook—Powder Metallurgy, vol. 7, 1997, pp. 14, 276, and 798.
- Petition for Inter Partes Review; Case No. IPR2017-00326; U.S. Pat. No. 9,101,978; Nov. 23, 2016; 46 pages.
- Petition for Inter Partes Review; Case No. IPR2017-00327; U.S. Pat. No. 8,573,295; Nov. 23, 2016; 53 pages.
- Schaffer, James P. et al.. The Science and Design of Engineering Materials, Second Edition, 1999, pp. 122, 123, 698, and 699.
- Xie, Guoqiang et al., "TEM Observation of Interfaces between Particles in Al-Mg Alloy Powder Compacts Prepared by Pulse Electric Current Sintering", Materials Transactions, 2002, pp. 2177-2180, vol. 43-No. 9.

\* cited by examiner

FIG. 1



FIG. 2A



FIG. 2B



FIG. 2C



## 1

**CORRODIBLE DOWNHOLE ARTICLE AND  
METHOD OF REMOVING THE ARTICLE  
FROM DOWNHOLE ENVIRONMENT**

**CROSS-REFERENCE TO RELATED  
APPLICATION**

This application is a division of U.S. patent application Ser. No. 13/162,781, filed Jun. 17, 2011, the disclosure of which is incorporated by reference herein in its entirety.

**BACKGROUND**

Certain downhole operations involve placement of elements in a downhole environment, where the element performs its function, and is then removed. For example, elements such as ball/ball seat assemblies and fracture (frac) plugs are downhole elements used to seal off lower zones in a borehole in order to carry out a hydraulic fracturing process (also referred to in the art as "fracking") to break up reservoir rock. After the fracturing operation, the ball/ball seat or plugs are then removed to allow fluid flow to or from the fractured rock.

To facilitate removal, such elements may be formed of a material that reacts with the ambient downhole environment so that they need not be physically removed by, for example, a mechanical operation, but may instead corrode or dissolve under downhole conditions. However, because operations such as fracturing may not be undertaken for months after the borehole is drilled, such elements may have to be immersed in downhole fluids for extended periods of time (for example, up to a year, or longer) before the fracturing operation begins. Therefore, it is desirable to have corrodible downhole elements such as ball seats and frac plugs that are protected from uncontrolled corrosion during that period of time, and which then can be subsequently made corrodible as needed.

**SUMMARY**

The above and other deficiencies of the prior art are overcome by a method of removing a corrodible downhole article having a surface coating, comprising eroding the surface coating by physical abrasion, chemical etching, or a combination of physical abrasion and chemical etching, the surface coating comprising a metallic layer of a metal resistant to corrosion by a corrosive material.

In another embodiment, a method of removing a corrodible downhole article which comprises a magnesium alloy core, and a metallic layer covering the magnesium alloy core, the metallic layer being resistant to corrosion by a corrosive material, the method comprising eroding the metallic layer by physical abrasion, chemical etching, or a combination of physical abrasion and chemical etching, and corroding the corrodible downhole article in a corrosive material after eroding.

In another embodiment, an article for forming a downhole seal comprises a magnesium alloy core, and a metallic layer having a thickness of about 100 to about 500 micrometers and covering the magnesium alloy core, the metallic layer being formed of nickel, aluminum, or an alloy thereof, and resistant to corrosion by a corrosive material, the article being a ball seat or frac plug.

In another embodiment, a method of making an article for forming a downhole seal, comprising plating, in the absence of water, a metallic layer having a thickness of about 100 to about 500 micrometers and resistant to corrosion by a

## 2

corrosive material, on a surface of a magnesium alloy core, the article being a ball seat or frac plug.

**BRIEF DESCRIPTION OF THE DRAWINGS**

5

Referring now to the drawings wherein like elements are numbered alike in the several Figures:

FIG. 1 shows a cross-sectional view of a corrodible downhole article 100 prior to removal of a protective coating 111 and seating of a ball 130; and

FIGS. 2A-2C show cross-sectional views of the sequential process for removing a protective coating 211 from a corrodible downhole article 200 (FIG. 2A), seating a ball 230 (FIG. 2B) in a seating zone 210 before fracturing, and removing the ball 230 and seating zone 210 after fracturing (FIG. 2C).

**DETAILED DESCRIPTION OF THE  
INVENTION**

20

A corrodible downhole article is disclosed, such as a ball seat or frac plug, where the downhole article includes a corrodible core, which dissolves in a corrosive environment, and a metallic layer covering the core. The metallic layer has sufficient thickness to resist scratching and premature erosion, but which is thin enough to be eroded physically, chemically, or by a combination including at least one of these types of processes prior to seating a ball on the ball seat. In this way, the seated core can be exposed to the corrosive downhole environment and the corrodible core corroded away to remove the article.

The corrodible downhole article, which is useful for forming a seal, includes a corrodible core that corrodes under downhole conditions, and a surface coating, which includes a metallic layer. The corrodible core has the surface coating on a surface of the core material.

The corrodible core comprises any material suitable for use in a downhole environment provided the core material is corrodible in the downhole environment. Core materials can include corrodible metals, metal oxides, composites, soluble glasses, and the like. Useful such core materials dissolve under aqueous conditions.

In an embodiment, the core material is a magnesium alloy. The magnesium alloy core includes magnesium or any magnesium alloy which is dissolvable in a corrosive environment including those typically encountered downhole, such as an aqueous environment which includes salt (i.e., brine), or an acidic or corrosive agent such as hydrogen sulfide, hydrochloric acid, or other such corrosive agents. Magnesium alloys suitable for use include alloys of magnesium with aluminum (Al), cadmium (Cd), calcium (Ca), cobalt (Co), copper (Cu), iron (Fe), manganese (Mn), nickel (Ni), silicon (Si), silver (Ag), strontium (Sr), thorium (Th), tungsten (W), zinc (Zn), zirconium (Zr), or a combination comprising at least one of these elements. Particularly useful alloys include magnesium alloy particles including those prepared from magnesium alloyed with Ni, W, Co, Cu, Fe, or other metals. Alloying or trace elements can be included in varying amounts to adjust the corrosion rate of the magnesium. For example, four of these elements (cadmium, calcium, silver, and zinc) have a mild-to-moderate accelerating effects on corrosion rates, whereas four others (copper, cobalt, iron, and nickel) have a still greater effect on corrosion. Exemplary commercial magnesium alloys which include different combinations of the above alloying elements to achieve different degrees of corrosion resistance include but are not limited to, for example, those alloyed

with aluminum, strontium, and manganese such as AJ62, AJ50x, AJ51x, and AJ52x alloys, and those alloyed with aluminum, zinc, and manganese such as AZ91A-E alloys.

It will be appreciated that alloys having corrosion rates greater than those of the above exemplary alloys are contemplated as being useful herein. For example, nickel has been found to be useful in decreasing the corrosion resistance (i.e., increasing the corrosion rate) of magnesium alloys when included in small amounts (i.e., less than 1% by weight). In an embodiment, the nickel content of a magnesium alloy is less than or equal to about 0.5 wt %, specifically less than or equal to about 0.4 wt %, and more specifically less than or equal to about 0.3 wt %, to provide a useful corrosion rate for the corrodible downhole article. In an exemplary embodiment, the magnesium particles are alloyed with about 0.25 wt % Ni.

The above magnesium alloys are useful for forming the core, and are formed into the desired shape and size by casting, forging and machining. Alternatively, powders of magnesium or the magnesium alloy are useful for forming the core. The magnesium alloy powder generally has a particle size of from about 50 to about 150 micrometers ( $\mu\text{m}$ ), and more specifically about 60 to about 140  $\mu\text{m}$ . The powder is further coated using a method such as chemical vapor deposition, anodization or the like, or admixed by physical method such cryo-milling, ball milling, or the like, with a metal or metal oxide such as Al, Ni, W, Co, Cu, Fe, oxides of one of these metals, or the like. Such coated magnesium powders are referred to herein as controlled electrolytic materials (CEM). The CEM materials are then molded or compressed into the desired shape by, for example, cold compression using an isostatic press at about 40 to about 80 ksi (about 275 to about 550 MPa), followed by forging or sintering and machining, to provide a core having the desired shape and dimensions.

It will be understood that the magnesium alloys, including CEM materials, will thus have any corrosion rate necessary to achieve the desired performance of the article. In a specific embodiment, the magnesium alloy or CEM material used to form the core has a corrosion rate of about 0.1 to about 20 mg/cm<sup>2</sup>/hour, specifically about 1 to about 15 mg/cm<sup>2</sup>/hour determined in aqueous 3 wt % KCl solution at 200° F. (93° C.).

The corrodible downhole article further has a surface coating, which includes a metallic layer. The metallic layer is resistant to corrosion by a corrosive material. As used herein, "resistant" means the metallic layer is not etched or dissolved by any corrosive downhole conditions encountered (i.e., brine, hydrogen sulfide, etc., at pressures greater than atmospheric pressure, and at temperatures in excess of 50° C.) such that any portion of the magnesium alloy core is exposed, for a period of greater than or equal to one year, specifically for a period of greater than or equal to two years.

The metallic layer includes any metal resistant to corrosion under ambient downhole conditions, and which can be removed by eroding as explained below. In an embodiment, the metallic layer includes nickel, aluminum, alloys thereof, or a combination comprising at least one of the foregoing. In an embodiment, the metallic layer is aluminum or aluminum alloy. In an embodiment, the metallic layer includes a single layer, or includes multiple layers of the same or different metals. In this way, the surface coating includes, in an embodiment, a metallic layer disposed on the core, and one or more additional layers of metal and/or metal oxide on the metallic layer. In an embodiment, adjacent, contacting layers in the surface coating have different compositions (e.g., are of different metals, combinations of metal and metal oxide,

etc.). Such outer layers may be formed by coating the metal layer with another metal, forming an oxide or anodized layer, or any such method of forming the outer layers.

The metallic layer has a thickness of less than or equal to about 1,000 micrometers (i.e., about 1 millimeter). In an embodiment, the metallic layer may have a thickness of about 10 to about 1,000 micrometers, specifically about 50 to about 750 micrometers and still more specifically about 100 to about 500 micrometers. The metallic layer covers a portion of the surface of the magnesium alloy core, or covers the entirety of the magnesium alloy core.

The metallic layer is applied to the corrodible core by any suitable method, provided that the application process is not carried out in the presence of agents which can react with the magnesium core, and which cause damage to the surface of the magnesium metal core, such that the desired properties of the metallic layer or magnesium alloy core are substantially adversely affected.

The metallic layer is thus formed by any suitable method for depositing a metal, including an electroless plating process, or by electrodeposition. Any suitable known method for applying the metallic layer can be used, provided the method does not significantly adversely affect the performance of the core after plating, such as by non-uniform plating or formation of surface defects affecting the integrity of the plated metallic layer on the magnesium alloy core.

Electroless deposition is useful for applying a uniform layer of metal over complex surface geometries. For example, the metal coating can be a nickel coating applied by an electroless process to the magnesium core such as that described by Ambat et al. (Rajan Ambat, W. Zhou, *Surf. And Coat. Technol.* 2004, vol. 179, pp. 124-134) or by Liu et al. (Zhenmin Liu, Wei Gao, *Surf. And Coat. Technol.* 2006, vol. 200, pp. 5087-93), the contents of both of which are incorporated herein by reference in their entirety.

In another embodiment, plating is carried out by electrodeposition in the presence of an anhydrous ionic solvent (i.e., in the absence of moisture). It will be appreciated that the presence of adventitious water during the plating process may cause surface pitting, or may cause formation of metal hydroxides, such as magnesium hydroxide, on the surface of the magnesium alloy core. Such surface defects may lead to a non-uniform adhesion of the metallic layer to the core, or may undesirably cause surface defects which can lead to weakened or compromised integrity of the metallic layer, hence reducing the effectiveness of the metallic layer in protecting the magnesium alloy core against corrosion.

A useful method of making an article thus includes plating the metallic layer in the absence of water, to form a metallic layer having a thickness of about 100 to about 500 micrometers and resistant to corrosion by a corrosive material, on a surface of a magnesium alloy core. For example, electrodeposition to apply an aluminum coating on a surface of a magnesium alloy can be carried out using, as a plating medium, aluminum chloride in 1-ethyl-3-methylimidazolium chloride as an ionic liquid, according to the literature method of Chang et al. (Jeng-Kuei Chang, Su-Yau Chen, Wen-Ta Tsai, Ming-Jay Deng, I-Wen Sun, *Electrochim. Comm.* 2007, vol. 9, pp. 1602-6), the contents of which are incorporated herein by reference in their entirety. In an embodiment, the article is a ball seat or frac plug.

Articles useful for downhole applications include ball seats and frac plugs. In an embodiment, the article has a generally cylindrical shape that tapers in a truncated, conical cross-sectional shape such as a ball seat, with an inside diameter in cylindrical cross-section of about 2 to about 15

cm, sufficient to allow, for example, a ball to fit downhole and to seat and form a seal in the desired downhole element. In a further embodiment, the surface is milled to have a concave region having a radius designed to accommodate a ball or plug.

In an embodiment, a method of removing the corrodible downhole article from a downhole environment includes eroding the surface coating of the article by physical abrasion, chemical etching, or a combination of physical abrasion and chemical etching, the surface coating being a metallic layer of a metal resistant to corrosion by a corrosive material. In another embodiment, the eroding is accomplished by physical abrasion alone.

Eroding comprises flowing a slurry of a proppant over the surface of the corrodible downhole article. A proppant includes any material useful for injecting into the fractured zones after the fracking process, to prop open the fractures in the downhole rock. Proppants useful herein have a hardness and abrasiveness greater than that of the surface layer. For example, useful proppants include sand including rounded sand grains, aluminum pellets, glass beads, ceramic beads including those based on alumina and zirconia, and the like, and combinations comprising at least one of the foregoing. In some embodiments, the proppant is polymer coated or is coated with a curable resin. Typical proppants have a mesh size of about 12 to about 70 mesh. The proppant is slurried in any suitable fluid used for fracking or other downhole fluid. For example, the fracking fluid includes distillate, diesel fuel, kerosene, polymer-based fluids, and aqueous fluids such as water, brine, dilute hydrochloric acid, or aqueous viscoelastic fluids such as those described in U.S. Pat. No. 7,723,272 which contains water, a viscoelastic surfactant (VES), additives to reduce viscosity (after delivery of the proppant), viscosity stabilizers and enhancers, and fluid loss control agents. A mixture of these fracking fluids with other solvents and/or surfactants commonly used in downhole applications is also useful herein.

Eroding includes partially or completely removing the metallic layer. Partial removal of the metallic layer during erosion, such as by wearing away patches, strips, or scratches which remove a portion of the surface of the metallic layer and which expose the underlying magnesium alloy, is in some embodiments sufficient to allow penetration of a corrosive material to and dissolution of the magnesium alloy. It will be appreciated that though physical abrasion by proppant is disclosed, the method is not limited to this. Abrasion may also be accomplished by other mechanical means, such as for example by insertion of a downhole tool or element and moving the tool or element with or against the corrodible downhole article to scratch or abrade the metallic layer.

The method further includes corroding the corrodible downhole article in a corrosive material after eroding. The corrosive material includes, for example, water, brine, an acid including hydrochloric acid, hydrogen sulfide, or a combination comprising at least one of the foregoing. In an embodiment, the corrosive material is injected downhole as a slurry containing the proppant, such as for example, a slurry of the proppant in brine, or is injected in a separate operation.

In another embodiment, a method of forming a reversible seal with a corrodible downhole article includes seating a ball or plug in the corrodible downhole article having a shaped surface, such as a concave shape, which accommodates a surface shape such as complementary a convex shape of the ball or plug, the corrodible downhole article comprising a magnesium alloy core, and a metallic layer covering

the magnesium alloy core. The metallic layer is resistant to corrosion by a corrosive material as described above. The downhole article prevents fluid flow further downhole when a ball or plug is seated in the downhole article.

5 Seating is accomplished by placing a ball or plug in the downhole environment, and applying pressure to the downhole environment to effect seating. Placing means, in the case of a ball seat, dropping a ball into the well pipe, and forcing the ball to settle to the ball seat by applying pressure. 10 As discussed above, the balls come in a variety of sizes scaled to seat with specific sized ball seats for isolating different fracture zones. For example, a lower fracture zone has a ball seat accommodating a smaller diameter ball than the ball seat for an upper fracture zone, so that the ball for sealing the lower fracture zone passes through the ball seat for the upper fracture zone, while the ball sized for the upper fracture zone seats on the upper fracture zone ball seat.

15 Forming the reversible seal further comprises removing the metallic layer of the corrodible downhole article, prior to seating, by injecting a slurry of a proppant into the downhole environment at a pressure greater than that of the downhole environment. During removing, the proppant slurry flows past the article and erodes the metallic layer to expose the magnesium alloy core to the downhole environment. In this 20 way, the ball or plug seats in the corrodible downhole article (e.g., ball seat) directly on the exposed magnesium alloy core.

25 Unseating of the corrodible downhole article can be accomplished by reducing the pressure applied to the downhole environment. This allows the pressure in the area below the seat to push up the seated ball, when the pressure applied to the downhole environment becomes less than that of the ambient downhole pressure.

30 In an embodiment, a method of removing a corrodible downhole article includes eroding the metallic layer by physical abrasion, chemical etching, or a combination of physical abrasion and chemical etching as described above, and corroding the corrodible downhole article in a corrosive material after eroding.

35 40 Removing the corrodible downhole article is accomplished by corroding the downhole article, after removal of at least a portion of the protective metallic layer, in a corrosive material present downhole. A useful corrosive material includes one of those described herein, and is included with the proppant, or is injected downhole after the proppant. For example, a slurry of a proppant in brine both 45 erodes the metallic layer and corrodes the magnesium alloy core. The abrasive action of the proppant erodes the metallic layer to expose all or a portion of the magnesium alloy core, and the exposed magnesium alloy core then corrodes in the brine of the proppant slurry.

50 The ball seat 100 is shown in schematic cross-section in FIG. 1. In FIG. 1, a ball seat 100 includes a surface coating layer 111 and magnesium alloy core 112 located in a seating zone 110 for accommodating a ball 130 (with the approximate location of the seated ball 130 shown by dashed lines). The narrowed seating zone 110 is within a housing 120, which is attached to a pipe or tube (not shown). The enclosure 120 has a composition different from that of the 55 magnesium alloy core 112. The ball seat 100, with ball 130 seated in seating zone 110 (after removal of the surface coating layer 111), closes off the lower (narrower) end of the ball seat 100 so that fracking is selectively carried out in the region above the seating zone 110.

60 65 In FIG. 2, the process of using the ball seat 200 is shown. In FIG. 2A, the ball seat 200 is shown prior to seating and fracking. A slurry of an abrasive material such as a proppant

or other abrasive material is passed into the fracking zone below the ball seat 200 (arrows showing direction of flow) through the seating zone 210, which erodes away all or a portion of the surface coating layer 211 to expose the magnesium alloy core 212. FIG. 2B shows the exposed magnesium alloy core 212, with a ball 230 seated in the seating zone 210 after the surface coating layer 211 has been removed by the action of the proppant. After fracking, the seated ball 230 and the magnesium alloy core 212 are exposed to a corrosive material, such as brine, which dissolves away the magnesium alloy core 212 (and hence seating zone 210). The ball 230 can be removed by dissolving while seated, or can first be unseated. FIG. 2C shows the ball seat 200 after removal (by dissolution) of the seating zone 210, where only housing 220 remains.

While one or more embodiments have been shown and described, modifications and substitutions may be made thereto without departing from the spirit and scope of the invention. Accordingly, it is to be understood that the present invention has been described by way of illustrations and not limitation.

All ranges disclosed herein are inclusive of the endpoints, and the endpoints are independently combinable with each other. The suffix "(s)" as used herein is intended to include both the singular and the plural of the term that it modifies, thereby including at least one of that term (e.g., the colorant (s) includes at least one colorants). "Optional" or "optionally" means that the subsequently described event or circumstance can or cannot occur, and that the description includes instances where the event occurs and instances where it does not. As used herein, "combination" is inclusive of blends, mixtures, alloys, reaction products, and the like. All references are incorporated herein by reference.

The use of the terms "a" and "an" and "the" and similar referents in the context of describing the invention (especially in the context of the following claims) are to be construed to cover both the singular and the plural, unless otherwise indicated herein or clearly contradicted by context. Further, it should further be noted that the terms "first," "second," and the like herein do not denote any order, quantity, or importance, but rather are used to distinguish one element from another. The modifier "about" used in connection with a quantity is inclusive of the stated value and has the meaning dictated by the context (e.g., it includes the degree of error associated with measurement of the particular quantity).

What is claimed is:

1. An article for forming a downhole seal, comprising a magnesium alloy core, and a metallic layer having a thickness of about 10 to about 1,000 micrometers and covering the magnesium alloy core, the metallic layer comprising tungsten, cobalt, copper, iron, nickel, aluminum, nickel alloy, aluminum alloy, or a combination comprising at least one of nickel, aluminum, nickel alloy, or aluminum alloy, and further the metallic layer being resistant to corrosion by a corrosive material, wherein the article is a ball seat; and a surface of the ball seat includes a concave region having a radius designed to accommodate a ball or plug.

2. The article of claim 1, wherein the magnesium alloy core comprises an alloy of magnesium with one or more of the following elements:

aluminum; cadmium; calcium; cobalt; copper; iron; manganese; nickel; silicon; silver; strontium; thorium; tungsten; zinc; or zirconium.

3. The article of claim 1, wherein the magnesium alloy article core comprises greater than zero but less than or equal to about 1 wt% of nickel.

4. The article of claim 1, wherein the magnesium alloy article core comprises about 0.25 to about 1 wt% of nickel.

5. The article of claim 1, wherein the metallic layer comprises one or more of the following: nickel; aluminum; nickel alloy; or aluminum alloy.

6. The article of claim 1, wherein the metallic layer comprises a single layer.

7. The article of claim 1, wherein the metallic layer comprises more than one layers.

10 8. The article of claim 5, wherein each of the metallic layer comprises different metals.

9. The article of claim 5, wherein each of the metallic layer comprises same metals.

15 10. The article of claim 1, wherein the metallic layer has a thickness of about 100 to about 500 micrometers.

11. A method of making an article for forming a downhole seal, comprising

plating or depositing, in the absence of water,

a metallic layer having a thickness of about 10 to about 1,000 micrometers and resistant to corrosion by a

corrosive material, on

a surface of a magnesium alloy core, wherein the metallic layer covers magnesium core and comprises tungsten, cobalt, copper, iron, nickel, aluminum, nickel alloy, aluminum alloy, or a combination comprising at least one of nickel, aluminum, nickel alloy, or aluminum alloy, the article is a ball seat, and a surface of the ball seat includes a concave region having a radius designed to accommodate a ball or plug.

30 12. The method of claim 11, wherein the metallic layer is formed by an electroless plating process, or by an electrodeposition process in the presence of an anhydrous ionic solvent.

13. The method of claim 11, further comprising forming the article core by forging, sintering, machining, or a combination comprising at least one of the foregoing.

14. The method of claim 13, comprising:

coating a powder to provide a coated powder;

molding or compressing the coated powder to provide a

molded or compressed article having a first shape; and

forming the article core by one or more of the following:

forging, sintering, or machining the molded or compressed article having the first shape.

15. The method of claim 14, wherein the powder has a

45 particle size of from about 50 to about 150 micrometers.

16. The method of claim 14, wherein the magnesium alloy article core comprises a powder having a particle size of from about 60 to about 140 micrometers.

50 17. The method of claim 11, wherein the metallic layer comprises one or more of the following: nickel; aluminum; nickel alloy; or aluminum alloy.

18. An article for forming a downhole seal, the article comprising:

a magnesium alloy article core, and

a metallic layer having a thickness of about 10 to about 1,000 micrometers and covering the magnesium alloy core, the metallic layer comprising tungsten, cobalt, copper, iron, nickel, aluminum, nickel alloy, aluminum alloy, or a combination comprising at least one of nickel, aluminum, nickel alloy, or aluminum alloy, and further the metallic layer being resistant to corrosion by a corrosive material,

wherein the article has a cylindrical shape that tapers in a truncated, conical cross- sectional shape.

55 19. The article of claim 18, wherein the magnesium alloy article core comprises particles of magnesium alloyed with one or more of the following: Ni; W; Co; Cu; or Fe.

**20.** The article of claim **18**, wherein the magnesium alloy article core comprises magnesium alloyed with less than or equal to about 0.5 wt% of nickel.

\* \* \* \* \*